



US006376166B1

(12) **United States Patent**  
Oya et al.

(10) **Patent No.:** US 6,376,166 B1  
(45) **Date of Patent:** Apr. 23, 2002

(54) **HEAT-DEVELOPABLE PHOTOSENSITIVE MATERIAL**

JP 60198540 10/1985  
JP 11288057 10/1999

(75) Inventors: **Toyohisa Oya; Katsuyuki Watanabe; Masaru Takasaki; Minoru Sakai, all of Minami-ashigara (JP)**

(73) Assignee: **Fuji Photo Film Co., Ltd., Kanagawa (JP)**

(\*) Notice: Subject to any disclaimer, the term of this patent is extended or adjusted under 35 U.S.C. 154(b) by 0 days.

(21) Appl. No.: **09/537,771**

(22) Filed: **Mar. 30, 2000**

(30) **Foreign Application Priority Data**

Mar. 30, 1999 (JP) ..... 11-090208  
Dec. 16, 1999 (JP) ..... 11-358136  
Jan. 31, 2000 (JP) ..... 2000-021209

(51) **Int. Cl.<sup>7</sup>** ..... **G03C 1/498**

(52) **U.S. Cl.** ..... **430/619**; 430/264; 430/543; 430/558; 430/613

(58) **Field of Search** ..... 430/619, 613, 430/264, 543, 558

(56) **References Cited**

**U.S. PATENT DOCUMENTS**

4,788,134 A \* 11/1988 Ozaki et al. ..... 430/619  
5,212,055 A \* 5/1993 Morigaki et al. ..... 430/551  
5,370,988 A \* 12/1994 Manganiello et al. ..... 430/619  
5,698,365 A \* 12/1997 Taguchi et al. ..... 430/203  
6,090,538 A \* 7/2000 Arai et al. ..... 430/619  
6,146,823 A \* 11/2000 Kato ..... 430/619

**FOREIGN PATENT DOCUMENTS**

JP 58149046 9/1983

**OTHER PUBLICATIONS**

The Theory of the Photographic Process, Fourth Edition, 1977, pp. 353-361.\*

\* cited by examiner

*Primary Examiner*—Thorl Chea

(74) *Attorney, Agent, or Firm*—Birch, Stewart, Kolasch & Birch, LLP

(57) **ABSTRACT**

A heat-developable photosensitive material which comprises, on the same side of a support, at least (a) a photosensitive silver halide, (b) a reducible silver salt, (c) a phenol compound represented by the following general formula (1), (d) a binder, and (e) a coupler compound:



wherein V<sup>1</sup> to V<sup>8</sup> each independently represent a hydrogen atom or a functional group; L represents a bridging group consisting of —CH(V<sup>9</sup>)— or —S—; V<sup>9</sup> represents a hydrogen atom or a functional group. The heat-developable photosensitive material causes extremely low fog and is suitable for photomechanical reproduction.

**18 Claims, 1 Drawing Sheet**

Fig. 1



# HEAT-DEVELOPABLE PHOTOSENSITIVE MATERIAL

## FIELD OF THE INVENTION

The present invention relates to a heat-developable photosensitive material, in particular, an ultrahigh contrast heat-developable photosensitive material. More specifically, the present invention relates to a heat-developable photosensitive material which causes almost no fog (Dmin), in particular, an ultrahigh contrast heat-developable photosensitive material which exhibits low Dmin and is suitable for photomechanical reproduction.

## BACKGROUND OF THE INVENTION

A large number of photosensitive materials are known which have a photosensitive layer on a support and form image by imaging exposure. An example of a system that enables environmental conservation or simplification of image formation includes a technique of forming an image by heat development.

In recent years, reduction of amount of waste processing solutions is strongly desired in the field of photomechanical processes from the standpoints of environmental protection and space savings. Techniques relating to photosensitive heat-developable photosensitive materials for use in photomechanical processes are required which enables efficient exposure by a laser scanner or a laser image setter and formation of a clear black image having high resolution and sharpness. Such photosensitive heat-developable materials can provide users with a simple and non-polluting heat development processing system that eliminates the use of solution-type processing chemicals.

Methods for forming an image by heat development are described, for example, in U.S. Pat. Nos. 3,152,904 and 3,457,075 and D. Morgan and B. Shely, *Imaging Processes and Materials, "Thermally Processed Silver Systems"* A, 8th ed., page 2, compiled by Sturge, V. Walworth and A. Shepp, Neblette (1969). The photosensitive material contains a reducible light-insensitive silver source (e.g., organic silver salt), a photocatalyst (e.g., silver halide) in a catalytically active amount, and a reducing agent for silver, which are usually dispersed in an organic binder matrix. This photosensitive material is stable at an ambient temperature, but when the material is heated at a high temperature (e.g., 8° C. or higher) after light exposure, silver is produced through an oxidation-reduction reaction between the reducible silver source (which functions as an oxidizing agent) and the reducing agent. The oxidation-reduction reaction is accelerated by catalytic action of a latent image generated upon exposure. The silver produced by the reaction of the reducible silver salt in the exposure region provides a black image and this presents a contrast to the non-exposure region to form an image.

Fog is a serious problem for heat-developable photosensitive materials. Various researches have been made to reduce the fog in silver halide photosensitive materials for thermal photography. As an antifogant, for example, U.S. Pat. No. 3,589,903 discloses use of mercury salts. Furthermore, there have also been disclosed uses of carboxylic acids such as benzoic acid and phthalic acid (U.S. Pat. No. 4,152,160), benzoylbenzoic acid compounds (U.S. Pat. No. 4,784,939), indane or tetralincarboxylic acids (U.S. Pat. No. 4,569,906), dicarboxylic acids (U.S. Pat. No. 4,820,617), heteroaromatic carboxylic acids (U.S. Pat. No. 4,626,500), halogenated compounds (U.S. Pat. Nos. 4,546,075, 4,756,999, 4,452,885, 3,874,946 and 3,955,982), halogen

molecules or halogen atoms bonded to heterocycles (U.S. Pat. No. 5,028,523), palladium compounds (U.S. Pat. No. 4,103,312 and British Patent No. 1,502,670), iron family compounds (U.S. Pat. No. 4,128,428), substituted triazoles (U.S. Pat. Nos. 4,123,374, 4,129,557 and 4,125,430), sulfur compounds (U.S. Pat. Nos. 4,213,784, 4,245,033, and JP-A-51-26019 [the abbreviation "JP-A" as used herein means an "unexamined published Japanese patent application"]), thiouracils (U.S. Pat. No. 4,002,479), sulfinic acid (JP-A-50-123331), metal salts of thiosulfonic acid (U.S. Pat. Nos. 4,125,403, 4,152,160 and 4,307,187), and combinations of metal salts of thiosulfonic acid and sulfinic acid (JP-A-53-20923 and JP-A-53-19825), thiosulfonic acid esters (JP-B-62-50810 [the abbreviation "JP-B" as used herein means an "examined Japanese patent publication"]], JP-A-7-209797 and JP-A-9-43760). There has also been disclosed use of disulphide compounds (JP-A-51-42529 and JP-B-63-37368).

However, those compounds have drawbacks, for example, insufficient anti-fog effect, decrease of Dmax and degraded image storage stability after development at a larger addition amount and so forth. Therefore, novel anti-fogants have been desired.

## SUMMARY OF THE INVENTION

In view of those drawbacks of the conventional materials and the existing need, an object of the present invention is to provide a heat-developable photosensitive material which causes extremely low fog (Dmin), in particular, an ultrahigh contrast heat-developable photosensitive material which exhibits low Dmin and is suitable for photomechanical reproduction.

The aforementioned object was achieved by the present invention. The present invention thus provides a heat-developable photosensitive material which comprises, on the same side of a support, at least (a) a photosensitive silver halide, (b) a reducible silver salt, (c) a phenol compound represented by the following general formula (1), (d) a binder, and (e) a coupler compound.



In the general formula (1), V<sup>1</sup> to V<sup>8</sup> each independently represent hydrogen atom or a functional group. L represents a bridging group consisting of —CH(V<sup>9</sup>)— or —S—. V<sup>9</sup> represents a hydrogen atom or a functional group.

The coupler compound used for the heat-developable photosensitive material of the present invention preferably consists of one or more of compounds represented by the following general formulae (2) to (14).





45 In the general formulae (2) to (14), X<sup>1</sup> to X<sup>15</sup> each independently represent a hydrogen atom or a functional group. In the general formula (2), R<sup>1</sup> and R<sup>2</sup> each independently represent an electron withdrawing group. In the general formulae (3) to (14), R<sup>3</sup> to R<sup>28</sup> each independently represent a hydrogen atom or a functional group. q represents an integer of 0-4.

50 (8) The heat-developable photosensitive material of the present invention preferably further comprises an ultrahigh contrast agent.

55 (5) According to the present invention, there can be provided a heat-developable photosensitive material causing almost no fog (Dmin) without degrading maximum density (Dmax) and sensitivity.

(9) 60 The symbol “-” used in the present specification indicates a range that includes the numerical values mentioned before and after the symbol.

#### BRIEF DESCRIPTION OF THE DRAWING

65 FIG. 1 is a side view of an exemplary heat developing apparatus used for the present invention. In the FIGURE, there are shown a heat-developable photosensitive material

10, carrying-in roller pairs 11, carrying-out roller pairs 12, rollers 13, a flat surface 14, heaters 15, and guide panels 16. The apparatus consists of a preheating section A, a heat developing section B, and a slow cooling section C.

## PREFERRED EMBODIMENT OF THE INVENTION

The heat-developable photosensitive material of present invention will be explained in detail below.

The heat-developable photosensitive material of the present invention comprises, on the same side of a support, an image-forming layer containing an organic silver salt as a reducible silver salt and a binder, and a photosensitive silver halide emulsion layer containing a photosensitive silver halide (photosensitive layer). The image-forming layer preferably contains a photosensitive silver halide and thereby functions also as the photosensitive layer. In addition, the heat-developable photosensitive material of the present invention comprises a particular phenol compound and coupler compound on the image-forming layer side, and thereby it can reduce fog (Dmin) to an extremely low level without degrading maximum image density (Dmax) and sensitivity.

The heat-developable photosensitive material of the present invention contains a phenol compound represented by the aforementioned general formula (1) on the same side of the support as the photosensitive silver halide and the reducible the silver salt.

In the general formula (1), V<sup>1</sup> to V<sup>8</sup> each independently represent a hydrogen atom or a functional group. In the present specification, the term "functional group" includes monovalent groups and atoms except for hydrogen atom. The functional groups represented by V<sup>1</sup> to V<sup>8</sup> may be the same or different from each other or one another. Preferred examples of the functional groups include a halogen atom (for example, fluorine atom, chlorine atom, bromine atom and iodine atom), a linear, branched or cyclic alkyl group having preferably 1–20 carbon atoms, more preferably 1–16 carbon atoms, further preferably 1–13 carbon atoms (for example, methyl, ethyl, n-propyl, isopropyl, sec-butyl, tert-butyl, tert-octyl, n-amyl, tert-amyl, n-dodecyl, n-tridecyl, cyclohexyl etc.), an alkenyl groups having preferably 2–20 carbon atoms, more preferably 2–16 carbon atoms, further preferably 2–12 carbon atoms (for example, vinyl, allyl, 2-but enyl, 3-pentenyl etc.), an aryl group having preferably 6–30 carbon atoms, more preferably 6–20 carbon atoms, further preferably 6–12 carbon atoms (for example, phenyl, p-methylphenyl, naphthyl etc.), an alkoxy group having preferably 1–20 carbon atoms, more preferably 1–16 carbon atoms, further preferably 1–12 carbon atoms (for example, methoxy, ethoxy, propoxy, butoxy etc.), an aryloxy group having preferably 6–30 carbon atoms, more preferably 6–20 carbon atoms, further preferably 6–12 carbon atoms (for example, phenoxy, 2-naphthoxy etc.), an acyloxy group having preferably 2–20 carbon atoms, more preferably 2–16 carbon atoms, further preferably 2–12 carbon atoms (for example, acetoxy, benzyloxy etc.), an amino group having preferably 0–20 carbon atoms, more preferably 1–16 carbon atoms, further preferably 1–12 carbon atoms (for example, dimethylamino group, diethylamino group, dibutylamino group, anilino group etc.), an acylamino group having preferably 2–20 carbon atoms, more preferably 2–16 carbon atoms, further preferably 2–13 carbon atoms (for example, acetyl amino, tridecanoyl amino, benzoyl amino etc.), a sulfonylamino group having preferably 1–20 carbon atoms, more preferably 1–16 carbon atoms, further preferably 1–12

carbon atoms (for example, methanesulfonylamino, butanesulfonylamino, benzenesulfonylamino etc.), a ureido group having preferably 1–20 carbon atoms, more preferably 1–16 carbon atoms, further preferably 1–12 carbon atoms (for example, ureido, methylureido, phenylureido etc.), a carbamate group having preferably 2–20 carbon atoms, more preferably 2–16 carbon atoms, further preferably 2–12 carbon atoms (for example, methoxycarbonylamino, phenyloxycarbonylamino etc.), a carboxyl group, a carbamoyl group having preferably 1–20 carbon atoms, more preferably 1–16 carbon atoms, further preferably 1–12 carbon atoms (for example, carbamoyl, N,N-diethylcarbamoyl, N-dodecylcarbamoyl, N-phenylcarbamoyl etc.), an alkoxy carbonyl group having preferably 2–20 carbon atoms, more preferably 2–16 carbon atoms, further preferably 2–12 carbon atoms (for example, methoxycarbonyl, ethoxycarbonyl, butoxycarbonyl etc.), an acyl group having preferably 2–20 carbon atoms, more preferably 2–16 carbon atoms, further preferably 2–12 carbon atoms (for example, acetyl, benzoyl, formyl, pivaloyl etc.), sulfo group, a sulfonyl group having preferably 1–20 carbon atoms, more preferably 1–16 carbon atoms, further preferably 1–12 carbon atoms (for example, mesyl, tosyl etc.), a sulfamoyl group having preferably 0–20 carbon atoms, more preferably 0–16 carbon atoms, further preferably 0–12 carbon atoms (for example, sulfamoyl, methylsulfamoyl, dimethylsulfamoyl, phenylsulfamoyl, etc.), cyano group, nitro group, hydroxyl group, mercapto group, an alkylthio group having preferably 1–20 carbon atoms, more preferably 1–16 carbon atoms, further preferably 1–12 carbon atoms (for example, methylthio, butylthio etc.), a heterocyclic group having preferably 2–20 carbon atoms, more preferably 2–16 carbon atoms, further preferably 2–12 carbon atoms (for example, pyridyl, imidazoyl, pyrrolidyl etc.). These functional groups may be further substituted with other functional groups.

Particularly preferred examples of the functional groups represented by  $V^1$  to  $V^8$  are alkyl groups (for example, methyl, ethyl, n-propyl, isopropyl, sec-butyl, tert-butyl, tert-octyl, n-amyl, tert-amyl, n-dodecyl, n-tridecyl, cyclohexyl etc.).

In the general formula (1), L represents a bridging group consisting of  $-\text{CH}(\text{V}^9)-$  or  $-\text{S}-$ .  $\text{V}^9$  represents a hydrogen atom or a functional group. Preferred examples of the functional group represented by  $\text{V}^9$  include, for example, a halogen atom (for example, fluorine atom, chlorine atom, bromine atom and an iodine atom), a linear, branched or cyclic alkyl group having preferably 1–20 carbon atoms, more preferably 1–16 carbon atoms, further preferably 1–13 45 carbon atoms (for example, methyl, ethyl, n-propyl, isopropyl, sec-butyl, tert-butyl, tert-octyl, n-amyl, tert-amyl, n-dodecyl, n-tridecyl, cyclohexyl, 2,4,4-trimethylpentyl etc.), an alkenyl groups having preferably 2–20 carbon atoms, more preferably 2–16 carbon atoms, further preferably 50 2–12 carbon atoms (for example, vinyl, allyl, 2-butenyl, 3-pentenyl etc.), an aryl group having preferably 6–30 carbon atoms, more preferably 6–20 carbon atoms, further preferably 6–12 carbon atoms (for example, phenyl, p-methylphenyl, naphthyl etc.), an alkoxy group having 55 preferably 1–20 carbon atoms, more preferably 1–16 carbon atoms, further preferably 1–12 carbon atoms (for example, methoxy, ethoxy, propoxy, butoxy etc.), an aryloxy group having preferably 6–30 carbon atoms, more preferably 6–20 carbon atoms, further preferably 6–12 carbon atoms (for 60 example, phenoxy, 2-naphthoxy etc.), an acyloxy group having preferably 2–20 carbon atoms, more preferably 2–16 carbon atoms, further preferably 2–12 carbon atoms (for 65 example, acetoxy, 2-naphthoacetoxy etc.).

example, acetoxy, benzyloxy etc.), an amino group having preferably 0–20 carbon atoms, more preferably 1–16 carbon atoms, further preferably 1–12 carbon atoms (for example, dimethylamino group, diethylamino group, dibutylamino group, anilino group etc.), an acylamino group having preferably 2–20 carbon atoms, more preferably 2–16 carbon atoms, further preferably 2–13 carbon atoms (for example, acetylamino, tridecanoylamino, benzoylamino etc.), a sulfonylamino group having preferably 1–20 carbon atoms, more preferably 1–16 carbon atoms, further preferably 1–12 carbon atoms (for example, methanesulfonylamino, butanesulfonylamino, benzenesulfonylamino etc.), a ureido group having preferably 1–20 carbon atoms, more preferably 1–16 carbon atoms, further preferably 1–12 carbon atoms (for example, ureido, methylureido, phenylureido etc.), a carbamate group having preferably 2–20 carbon atoms, more preferably 2–16 carbon atoms, further preferably 2–12 carbon atoms (for example, methoxycarbonylamino, phenoxy carbonylamino etc.), carboxyl group, a carbamoyl group having preferably 1–20 carbon atoms, more preferably 1–16 carbon atoms, further preferably 1–12 carbon atoms (for example, carbamoyl, 25 N,N-diethylcarbamoyl, N-dodecylcarbamoyl, N-phenylcarbamoyl etc.), an alkoxy carbonyl group having preferably 2–20 carbon atoms, more preferably 2–16 carbon atoms, further preferably 2–12 carbon atoms (for example, methoxycarbonyl, ethoxycarbonyl, butoxycarbonyl etc.), an 30 acyl group having preferably 2–20 carbon atoms, more preferably 2–16 carbon atoms, further preferably 2–12 carbon atoms (for example, acetyl, benzoyl, formyl, pivaloyl etc.), sulfo group, a sulfonyl group having preferably 1–20 carbon atoms, more preferably 1–16 carbon atoms, further 35 preferably 1–12 carbon atoms (for example, mesyl, tosyl etc.), a sulfamoyl group having preferably 0–20 carbon atoms, more preferably 0–16 carbon atoms, further preferably 0–12 carbon atoms (for example, sulfamoyl, 40 methylsulfamoyl, dimethylsulfamoyl, phenylsulfamoyl, etc.), cyano group, nitro group, hydroxyl group, mercapto group, an alkylthio group having preferably 1–20 carbon atoms, more preferably 1–16 carbon atoms, further 45 preferably 1–12 carbon atoms (for example, methylthio, butylthio etc.), a heterocyclic group having preferably 2–20 carbon atoms, more preferably 2–16 carbon atoms, further preferably 2–12 carbon atoms (for example, pyridyl, imidazoyl, 50 pyrrolidyl etc.). These functional groups may be further substituted with other functional groups.

Particularly preferred examples of the functional group represented by  $V^9$  are an alkyl group (for example, methyl, ethyl, n-propyl, isopropyl, sec-butyl, tert-butyl, tert-octyl, 55 n-amyl, n-octyl, tert-amyl, n-dodecyl, n-tridecyl, cyclohexyl, 2,4,4-trimethylpentyl etc.), an alkenyl group (for example, vinyl, allyl, 2-but enyl, 3-pentenyl etc.), an aryl group (for example, phenyl, p-methylphenyl, naphthyl etc.), 60 hydroxyl group, mercapto group, an alkylthio group (for example, methylthio, butylthio etc.) and so forth.

Specific examples of the phenol compound represented by the general formula (1) will be shown below. However, the 65 scope of the phenol compound used for the present invention is not limited to these examples.



(I-1)



(I-2)



(I-3)



(I-4)



(I-5)



(I-6)

**9**

-continued

**10**

-continued



**11**

-continued

**12**

-continued



13

-continued



(I-33)



(I-34)

The amount of the phenol compound represented by the formula (1) used for the present invention is preferably 0.01 to 4.0 g, more preferably 0.2 to 2.0 g, further preferably 0.5 to 2.0 g per 1 m<sup>2</sup> of the photosensitive material. Further, it is preferably contained in an amount of 5 to 500 mmol, more preferably 10 to 400 mmol per mole of silver present on the surface having the image-forming layer.

The phenol compound used for the present invention may be added in any form, for example, as a solution, powder, solid fine grain dispersion and so forth. The solid fine grain dispersion can be formed by a known pulverization means (for example, a ball mill, a vibration ball mill, a sand mill, a colloid mill, a jet mill, a roller mill etc.). Further, when a solid fine grain dispersion is prepared, a dispersing aid may be used.

The phenol compound used for the present invention may be added to any layers on a support provided on the same side as layers containing the aforementioned photosensitive silver halide and the reducible silver salt are present. However, it is preferably added to a layer containing the silver halide or a layer adjacent thereto.

The heat developable photosensitive material of the present invention contains a coupler compound on the same said of a support as the surface provided with the aforementioned photosensitive silver halide and the reducible silver salt. As a two equivalent or four equivalent coupler compound used for the present invention, two equivalent or four equivalent couplers well known in the photographic industry can be used. Inter alia, it is preferable to use one or more compounds represented by the aforementioned general formulae (2) to (14).

In the general formula (2) to (14), X<sup>1</sup> to X<sup>15</sup> each independently represent a hydrogen atom or a functional group. The functional groups represented by X<sup>1</sup> to X<sup>15</sup> may be the same or different from each other or one another. Preferred examples of the functional groups include a halogen atom (for example, fluorine atom, chlorine atom, bromine atom and iodine atom), an aryl group having preferably 6-30 carbon atoms, more preferably 6-20 carbon atoms, further preferably 6-12 carbon atoms (for example, phenyl, p-methylphenyl, naphthyl etc.), an alkoxy group having preferably 1-20 carbon atoms, more preferably 1-12 carbon atoms, further preferably 1-8 carbon atoms (for example, methoxy, ethoxy, butoxy etc.), an aryloxy group having preferably 6-20 carbon atoms, more preferably 6-16 carbon

14

atoms, further preferably 6-12 carbon atoms (for example, phenyloxy, 2-naphthyoxy etc.), an alkylthio group having preferably 1-20 carbon atoms, more preferably 1-16 carbon atoms, further preferably 1-12 carbon atoms (for example, methylthio, ethylthio, butylthio etc.), an arylthio group having preferably 6-20 carbon atoms, more preferably 6-16 carbon atoms, further preferably 6-12 carbon atoms (for example, phenylthio, naphthylthio etc.), an acyloxy group having preferably 1-20 carbon atoms, more preferably 2-16 carbon atoms, further preferably 2-10 carbon atoms (for example, acetoxy, benzyloxy etc.), an acylamino group having preferably 2-20 carbon atoms, more preferably 2-16 carbon atoms, further preferably 2-10 carbon atoms (for example, N-methylacetylarnino, benzoylarnino etc.), a sulfonylarnino group having preferably 1-20 carbon atoms, more preferably 1-16 carbon atoms, further preferably 1-12 carbon atoms (for example, methanesulfonylarnino, benzene-sulfonylarnino etc.), a carbamoyl group having preferably 1-20 carbon atoms, more preferably 1-16 carbon atoms, further preferably 1-12 carbon atoms (for example, carbamoyl, N,N-diethylcarbamoyl, N-phenylcarbamoyl, etc.), an acyl group having preferably 2-20 carbon atoms, more preferably 2-16 carbon atoms, further preferably 2-12 carbon atoms (for example, acetyl, benzoyl, formyl, pivaloyl etc.), an alkoxy carbonyl group having preferably 2-20 carbon atoms, more preferably 2-16 carbon atoms, further preferably 2-12 carbon atoms (for example, methoxycarbonyl etc.), sulfo group, a sulfonyl group having preferably 1-20 carbon atoms, more preferably 1-16 carbon atoms, further preferably 1-12 carbon atoms (for mesyl, tosyl etc.), a sulfonyloxy group having preferably 1-20 carbon atoms, more preferably 1-16 carbon atoms, further preferably 1-12 carbon atoms (for example, methanesulfonyloxy, benzene-sulfonyloxy etc.), azo group, a heterocyclic group, a heterocyclylmercapto group, cyano group and so forth. The heterocyclic group herein used refers to a saturated or unsaturated heterocyclic group, and examples thereof include, for example, pyridyl group, quinolyl group, quinoxalinyl group, pyrazinyl group, benzotriazolyl group, pyrazolyl group, imidazolyl group, benzimidazolyl group, tetrazolyl group, hydantoin-1-yl group, succinimide group, phthalimide group and so forth. These functional groups may be further substituted with other functional groups. Such functional groups may be any of generally known functional groups so long as they do not degrade photographic performance.

The functional groups represented by X<sup>1</sup> to X<sup>15</sup> are preferably those known as releasing groups of two equivalent photographic couplers, and examples thereof include, for example, hydrogen atom, a halogen atom, an alkoxy group, an aryloxy group, an alkylthio group, an arylthio group, a heterocyclic group, a heterocyclylmercapto group and so forth.

In the general formula (2), R<sup>1</sup> and R<sup>2</sup> may be the same or different from each other, and they represent an electron withdrawing group. The electron withdrawing group herein used means a functional group having a Hammett's functional group constant  $\sigma_p$  of a positive value, and specific examples thereof include cyano group, an alkoxy carbonyl group, an aryloxy carbonyl group, a carbamoyl group, imino group, an imino group substituted at N atom, a thiocarbonyl group, a sulfamoyl group, an alkylsulfonyl group, an arylsulfonyl group, nitro group, a halogen atom, a perfluoroalkyl group, a perfluoroalkane amide group, a sulfonamide group, an acyl group, benzoyl group, formyl group, phosphoryl group, carboxy group (or a salt thereof), formyl group, phosphoryl group, carboxy group (or a salt thereof), sulfo

15

group (or a salt thereof), a heterocyclic group, an alkenyl group, an alkynyl group, an acyloxy group, an acylthio group, a sulfonyloxy group, an aryl group which is substituted with one or more of these electron withdrawing groups and so forth. Examples of the heterocyclic group include saturated or unsaturated heterocyclic groups, for example, pyridyl group, quinolyl group, quinoxaliny group, pyrazinyl group, benzotriazolyl group, imidazolyl group, benzimidazolyl group, hydantoin-1-yl group, succinimide group, phthalimide group, indolinyl and so forth. Moreover, R<sup>1</sup> and R<sup>2</sup> may be bonded together to form a saturated or unsaturated carbon ring or heterocyclic ring. In particular, preferred are those functional groups having 30 carbon atoms or less, more preferably 20 carbon atoms or less. More preferably, they represent cyano group, an alkoxy carbonyl group, an aryloxy carbonyl group, a carbamoyl group, an imino group, an acyl group, benzoyl group or a heterocyclic group.

In the general formulae (3) to (14), R<sup>3</sup> to R<sup>28</sup> each independently represent a hydrogen atom or a functional group. The functional groups represented by R<sup>3</sup> to R<sup>28</sup> may be the same or different from one another, and any functional groups may be used so long as they do not degrade photographic performance. Specific examples thereof include those functional groups mentioned as preferred examples of V<sup>1</sup> to V<sup>8</sup>. Those functional groups may be further substituted with other functional groups. Moreover, when q is 2 or higher number and there are two or more adjacent R<sup>27</sup>, two adjacent R<sup>27</sup> may form a ring.

Preferred examples of the functional groups represented by R<sup>3</sup> to R<sup>28</sup> are a halogen atom, an alkyl group, an aryl group, an alkoxy group, an aryloxy group, an acyloxy group, an anilino group, an acylamino group, a sulfonylamino group, carboxyl group, a carbamoyl group, an acyl group, sulfo group, a sulfonyl group, a sulfamoyl group, cyano group, hydroxyl group, mercapto group, an alkylthio group and a heterocyclic group.

In the heat-developable photosensitive material of the present invention, while the compound represented by the general formulae (2) to (16) are preferred as the coupler compound, compounds represented by the general formulae (2), (4), (5), (7), (8), (9), (10) and (14) are more preferred, and the compounds represented by the general formulae (4), (5), (8), (9) and (10) are particularly preferred.

Specific examples of the compounds represented by the general formulae (2) to (14) are listed below. However, the coupler compound used for the present invention is not limited to these.



(A-101)

55



(A-102)

60



(A-103)

65

16  
-continued

(A-104)



(A-105)



(A-106)



(A-107)



(A-108)



(A-109)



(A-110)



(A-111)



17

-continued



(A-112)

5

(A-113) 15



25



35



(A-204) 50



(A-205)

18

-continued



(A-206)



(A-207)



(A=208)



(A-209)



(A-301)



60



(A-303)



5

10

15

(A-308)



(A-304)



20

25

(A-309)



(A-305)



35

40

(A-310)



(A-306)



45

50

(A-311)



(A-307)



55

60

**21**

-continued

**22**

-continued

(A-312)



5

(A-401)



10

(A-402)



20

(A-403)



25

(A-404)



30

35

40

45

50

55

60

65

(A-405)

(A-406)

(A-407)

(A-408)

(A-409)

**23**

-continued

**24**

-continued

(A-501)



5 (A-502)

10

(A-503)

15

20

25

(A-504)

30

35

(A-505)

40

(A-506)

45

50

55

60



(A-507)

(A-508)

(A-601)

(A-602)

(A-603)

25

-continued



(A-604)

5



(A-903)



(A-605)

15



(xx-666)

30



(A-906)



(A-607) 40

45



(A-908)



55



(A-909)



(A-222)





**29**

-continued

**30**

-continued

(A-1012)



5

(A-1013)



10

(A-1014)



20

(A-1101)



30

(A-1102)



35

(A-1103)



40

(A-1104)



45

(A-1105)



50

(A-1106)

(A-1106)



(A-1107)



(A-1108)



(A-1109)



(A-1110)



(A-1111)



(A-1112)



(A-1113)



60

65

**31**

-continued

**32**

-continued

(A-1114)



(A-1115)



(A-1201)



(A-1202)



(A-1204)



(A-1205)

(A-1206)

(A-1207)

(A-1208)

(A-1209)

**33**

-continued

**34**

-continued

(A-1301)



(A-1302)



(A-1303)



(A-1304)



(A-1305)



(A-1306)



(A-1307)

(A-1308)

(A-1309)

(A-1310)

(A-1401)

35

-continued



36

-continued

(A-1501)



65



(A-1403) 1



1



(A-1404)



(A-1405)



(A-1406)



4



4.



(A-1409)

60 The coupler compounds represented by the general formulae (2) to (14), which are preferably used for the present invention, can readily be synthesized by methods known in the photographic industry.

65 The amount of the coupler compound used for the present invention is preferably 0.2 to 200 mmol, more preferably 0.3 to 100 mmol, further preferably 0.5 to 30 mmol, per mole of

silver. Each of the coupler compounds may be used alone, or they may be used in a combination of two or more of them.

The coupler compound used for the present invention may be used by dissolving said compound in water or a suitable organic solvent, for example, alcohols such as methanol, ethanol, propanol and fluorinated alcohol, ketones such as acetone and methyl ethyl ketone, dimethylformamide, dimethyl sulfoxide, methyl cellosolve and the like. Alternatively, the compound may also be used as an emulsified dispersion mechanically prepared according to an already well known emulsification dispersion method by using an oil such as dibutyl phthalate, tricresyl phosphate, glyceryl triacetate or diethyl phthalate, ethyl acetate or cyclohexanone as an auxiliary solvent for dissolution. Alternatively, the compounds may be used after dispersion of a powder in water by using a ball mill, a colloid mill, a sand grinder mil, MANTON GAULIN, a microfluidizer, or by means of ultrasonic wave according to a known method for solid dispersion.

The coupler compound used for the present invention may be added to any layers on a support provided that the layers are present on the side of the support which has a layer or layers containing the aforementioned photosensitive silver halide and the reducible silver salt. However, it is preferably added to a layer containing the silver halide or a layer adjacent thereto.

The photosensitive silver halide for use in the present invention is not particularly limited as for the halogen composition, and silver chloride, silver chlorobromide, silver bromide, silver iodobromide, and silver chloroiodobromide may be used.

The halide composition may have a uniform distribution in the grains, or the compositions may change stepwise or continuously in the grains. Silver halide grains having a core/shell structure may be preferably used. Core/shell grains having preferably a double to quintuple structure, more preferably a double to quadruple structure may be used. A technique for localizing silver bromide on silver halide or silver chlorobromide may also be preferably used.

For the preparation of the photosensitive silver halide used for the present invention, methods well known in the art, e.g., the methods described in Research Disclosure, No. 17029 (June, 1978) and U.S. Pat. No. 3,700,458, can be used. More specifically, applicable methods for the present invention include a method comprising the step of adding a halogen-containing compound to a ready prepared organic silver salt to convert a part of silver of the organic silver salt into a photosensitive silver halide, and a method comprising the step of preparing photosensitive silver halide grains by adding a silver-supplying compound and a halogen-supplying compound to a solution of gelatin or another polymer and then mixing the prepared grains with an organic silver salt. In particular, the latter method is preferred for the present invention.

As for a grain size of the photosensitive silver halide, smaller grains are desirable to prevent cloudiness of the photosensitive material after image formation. Specifically, the grain size may preferably be not greater than  $0.20 \mu\text{m}$ , preferably from  $0.01$  to  $0.15 \mu\text{m}$ , more preferably from  $0.02$  to  $0.12 \mu\text{m}$ . The term "grain size" used herein means "ridge length" of silver halide grains when the silver halide grains are regular crystals in cubic or octahedral form. Where silver halide grains are tabular grains, the term means the diameter of a circle having the same area as a projected area of the main surface of the tabular grain. Where the silver halide grains are irregular crystals, such as spherical or rod-like

grains, the term means the diameter of a sphere having the same volume as the grain.

Examples of the form of silver halide grains include a cubic form, octahedral form, tabular form, spherical form, rod-like form and potato-like form. In particular, cubic grains and tabular grains are preferred for the present invention. When tabular silver halide grains are used, an average aspect ratio may be from  $100:1$  to  $2:1$ , preferably from  $50:1$  to  $3:1$ . Silver halide grains having round corners are also preferably used in the present invention.

Surface index (Miller index) of outer surfaces of the photosensitive silver halide grains is not particularly limited. However, it is desirable that [100] face be present in a high proportion which can achieve high spectral sensitizing efficiency when a spectral sensitizing dye adsorbed thereto. The proportion of [100] face may be not lower than  $50\%$ , preferably at least  $65\%$ , and more preferably at least  $80\%$ . The proportion of [100] face can be determined using the method described in T. Tani, J. Imaging Sci., 29, 165 (1985), where the difference in adsorption of a sensitizing dye to [111] face and [100] face is utilized.

The silver halide emulsion may be used alone in the photosensitive material of the present invention, or two or more of them may be used in combination (for example, those having different average grain sizes, different halogen compositions, or different crystallization properties, or those produces under different sensitization conditions).

The amount of the photosensitive silver halide used in the present invention may preferably be from  $0.01$  to  $0.5 \text{ mol}$ , more preferably from  $0.02$  to  $0.3 \text{ mol}$ , and more preferably from  $0.03$  to  $0.25 \text{ mol}$  based on per mole of the reducible silver salt.

The photosensitive silver halide for use in the present invention preferably contains a metal of Group VII or VIII (group 7 to 10) in the periodic table of elements, metal compound or metal complex thereof. The metal of Group VII or VIII of the periodic table or center metal of the metal compound and metal complex thereof is preferably rhodium, rhenium, ruthenium, osmium or iridium. More specifically, the metal complexes having the structures described in JP-A-7-225449 may be used. These metals and the metal complexes may be used alone, or two or more of them may be used in combination, or two or more complexes with the same or different metals may also be used in combination.

The content of metals of Group VII or VIII of the periodic table, metal compounds and metal complexes thereof is preferably from  $1 \times 10^{-9}$  to  $1 \times 10^{-2} \text{ mol}$ , more preferably from  $1 \times 10^{-8}$  to  $1 \times 10^{-4} \text{ mol}$  based on one mole of silver halide.

As the rhodium compound, a water-soluble rhodium compound may be used. Examples include a rhodium(III) halogenide compounds and rhodium complex salts having a halogen, an amine or an oxalate as a ligand, such as hexachlororhodium(III) complex salt, pentachloroaurorhodium(III) complex salt, tetrachlororhodium(III) complex salt, hexabromorhodium(III) complex salt, hexaamminorhodium(III) complex salt and trioxalatorhodium(III) complex salt.

The rhodium compound is used after being dissolved in water or an appropriate solvent, and a method commonly used for stabilizing the rhodium compound solution may be applied, for example, a method comprising the step of adding an aqueous solution of hydrogen halide (e.g., hydrochloric acid, hydrobromic acid, hydrofluoric acid) or alkali metal halide (e.g., KCl, NaCl, KBr, NaBr) may be used. Instead of the use of a water-soluble rhodium, different

silver halide grains doped beforehand with rhodium may be added and dissolved at the time of preparation of silver halide.

The amount of the rhodium compound is preferably from  $1 \times 10^{-8}$  to  $5 \times 10^{-6}$  mol, more preferably from  $5 \times 10^{-8}$  to  $1 \times 10^{-6}$  mol based on one mole of silver halide.

The rhenium, ruthenium or osmium is added in the form of a water-soluble complex salt described in JP-A-63-2042, JP-A-1-285941, JP-A-2-20852 and JP-A-2-20855. Particularly preferred examples are six-coordinate complex salts represented by the following formula:



wherein M represents Ru, Re or Os, L represents a ligand, and n represents 0, 1, 2, 3 or 4.

In this case, the counter ion plays no important role and an ammonium or alkali metal may be used.

Preferred examples of the ligand represented by L include a halide ligand, a cyanide ligand, a cyan oxide ligand, a nitrosyl ligand, a thionitrosyl ligand and the like. Specific examples of the complex for use in the present invention are shown below. However, the scope of the present invention is not limited to these examples.

|                       |                        |                        |
|-----------------------|------------------------|------------------------|
| $[ReCl_6]^{3-}$       | $[ReBr_6]^{3-}$        | $[ReCl_5(NO)]^{2-}$    |
| $[Re(NS)Br_5]^{2-}$   | $[Re(NO)(CN)_5]^{2-}$  | $[Re(O)_2(CN)_4]^{3-}$ |
| $[RuCl_6]^{3-}$       | $[RuCl_4(H_2O)_2]^{+}$ | $[RuCl_5(H_2O)]^{2-}$  |
| $[RuCl_5(NO)]^{2-}$   | $[RuBr_5(NS)]^{2-}$    |                        |
| $[Ru(CO)_3Cl_3]^{2-}$ | $[Ru(CO)Cl_5]^{2-}$    | $[Ru(CO)Br_5]^{2-}$    |
| $[OsCl_6]^{3-}$       | $[OsCl_5(NO)]^{2-}$    | $[Os(NO)(CN)_5]^{2-}$  |
| $[Os(NS)Br_5]^{2-}$   | $[Os(O)_2(CN)_4]^{4-}$ |                        |

The amount of rhenium, ruthenium or osmium or these compounds is preferably from  $1 \times 10^{-9}$  to  $1 \times 10^{-5}$  mol, most preferably from  $1 \times 10^{-8}$  to  $1 \times 10^{-6}$  mol based on one mole of silver.

As the iridium compound, various compounds may be used. Examples include hexachloroiridium, hexammineiridium, trioxalatoiridium, hexacyanoiridium, pentachloronitrosyliridium and the like.

Those iridium compounds are used after being dissolved in water or an appropriate solvent, and a method commonly used for stabilizing the iridium compound solution, more specifically, a method comprising the step of adding an aqueous solution of hydrogen halide (e.g., hydrochloric acid, bromic acid, hydrofluoric acid) or alkali metal halide (e.g., KCl, NaCl, KBr, NaBr) may be used. Instead of using a water-soluble iridium, different silver halide grains doped beforehand with iridium may be added and dissolved at the time of preparation of silver halide.

The metals of Group VII or VIII, metal compounds and metal complexes thereof may be added appropriately at the time of preparation of silver halide emulsion grains or at each stages before the coating of the emulsion. The compounds are preferably added at the time of formation of the emulsion and incorporated into silver halide grains.

For the addition of the compound during the grain formation of silver halide for incorporation in silver halide grains, examples of applicable methods include, for example, a method where a metal complex powder or an aqueous solution of the complex dissolved with NaCl or KCl is added to a water-soluble salt or water-soluble halide solution during the grain formation, a method where the compound is added as a "third" solution at the time of simultaneous mixing of a silver salt and a halide solution to prepare silver halide grains by the simultaneous mixing of

the three solutions, or a method where a necessary amount of an aqueous metal complex solution is poured into a reaction vessel during the grain formation. Among these, the method is preferred which comprises the step of adding a metal complex powder or an aqueous solution of the complex dissolved with NaCl or KCl to a water-soluble halide solution.

In order to add the compounds to the surface of the grain, a necessary amount of an aqueous metal complex solution may be charged into a reaction vessel immediately after the grain formation, during or after completion of the physical ripening, or at the time of chemical ripening.

The silver halide for use in the present invention may further contain a metal atom such as cobalt, iron, nickel, chromium, palladium, platinum, gold, thallium, copper and lead. In the case of cobalt, iron, chromium or ruthenium compound, a hexacyano metal complex is preferably used. Specific examples include ferricyanide ion, ferrocyanate ion, hexacyanocobaltate ion, hexacyanochromate ion and hexacyanoruthenate ion. However, the present invention is not limited to these examples.

The above-described metal is used preferably in an amount of from  $1 \times 10^{-9}$  to  $1 \times 10^{-4}$  mol based on one mole of silver halide. The metal may be converted into a metal salt in the form of a simple salt, a composite salt or a complex salt, and added at the time of preparation of silver halide grains. The metal complex may be added, for example, uniformly in the silver halide, added in a higher concentration in the core part or in the shell part, and a way of the addition of the metal complex is not particularly limited.

In the silver halide for use in the present invention, a cadmium salt, sulfite, lead salt or thallium salt may be allowed to coexist during the formation or physical ripening of the silver halide grains.

To the silver halide, a thiosulfonic acid compound may be added by the method described in European Patent 293917A.

The photosensitive silver halide grain used for the present invention may be desalts by water washing according to a method known in the art, such as noodle washing and flocculation. However, the grain may not be desalts in the present invention.

The silver halide emulsion for use in the present invention is preferably subjected to chemical sensitization. The chemical sensitization may be performed using a known method such as sulfur sensitization, selenium sensitization, tellurium sensitization, noble metal sensitization and reduction sensitization. These sensitization method may be used alone or in any combination. When these sensitization methods are used in combination, a combination of sulfur sensitization and gold sensitization, a combination of sulfur sensitization, selenium sensitization and gold sensitization, a combination of sulfur sensitization, tellurium sensitization and gold sensitization, and a combination of sulfur sensitization, selenium sensitization, tellurium sensitization and gold sensitization, for example, are preferred.

The sulfur sensitization is usually performed by adding a sulfur sensitizer and stirring the emulsion at a high temperature of  $40^{\circ}\text{C}$ . or higher for a given time. A known compound may be used as the sulfur sensitizer, and examples include a sulfur compound contained in gelatin, as well as various sulfur compounds such as thiosulfates, thioureas, thiazoles and rhodanines. Preferred sulfur compounds are thiosulfate and thiourea compounds. The amount of the sulfur sensitizer varies depending on various conditions such as pH and a temperature at the chemical ripening and the size of silver halide grain. A preferred amount may be from  $10^{-7}$  to  $10^{-2}$

mol, more preferably from  $10^{-5}$  to  $10^{-3}$  mol based on one mole of silver halide.

As the selenium sensitizer for use in the selenium sensitization, a known selenium compound may be used. The selenium sensitization is usually performed by adding a labile and/or non-labile selenium compound and stirring the emulsion at a high temperature of 40° C. or higher for a given time. Examples of the labile selenium compound include the compounds described in JP-B-44-15748, JP-B-43-13489, JP-A-4-25832, JP-A-4-109240 and JP-A-4-324855. Among them, particularly preferred compounds are those represented by formulae (VIII) and (IX) of JP-A-4-324855.

The tellurium sensitizer for use in the tellurium sensitization is a compound of forming silver telluride, presumably working as a sensitization nucleus, on the surface or inside of a silver halide grain. The rate of the formation of silver telluride in a silver halide emulsion can be examined according to a method described in JP-A-5-313284. Examples of the tellurium sensitizer include diacyl tellurides, bis(oxycarbonyl) tellurides, bis(carbamoyl) tellurides, diacyl tellurides, bis(oxycarbonyl) ditellurides, bis(carbamoyl) ditellurides, compounds having a P—Te bond, tellurocarboxylates, Te-organyltellurocarboxylic acid esters, di(poly)tellurides, tellurides, tellurols, telluroacetals, tellurosulfonates, compounds having a P—Te bond, Te-containing heterocyclic rings, tellurocarbonyl compounds, inorganic tellurium compounds, colloidal tellurium and the like. Specific examples thereof include the compounds described in U.S. Pat. Nos. 1,623,499, 3,320, 069 and 3,772,031, British Patent Nos. 235,211, 1,121,496, 1,295,462 and 1,396,696, Canadian Patent No. 800,958, JP-A-4-204640, JP-A-5-303157, J. Chem. Soc. Chem. Commun., 635 (1980), ibid., 1102 (1979), ibid., 645 (1979), J. Chem. Soc. Perkin. Trans., 1, 2191 (1980), S. Patai (compiler), The Chemistry of Organic Selenium and Tellurium Compounds, Vol. 1 (1986), and ibid., Vol. 2 (1987) and the like. The compounds represented by formulae (II), (III) and (IV) of JP-A-5-313284 are particularly preferred.

The amount of the selenium or tellurium sensitizer varies depending on silver halide grains used, chemical ripening conditions or the like. However, it is usually from  $1 \times 10^{-8}$  to  $1 \times 10^{-2}$  mol, preferably from  $1 \times 10^{-7}$  to  $1 \times 10^{-3}$  mol based on one mole of silver halide. The conditions for chemical sensitization in the present invention are not particularly limited. In general, pH of from 5 to 8, pAg of from 6 to 11, preferably from 7 to 10 may be applied, and a temperature may be from 40 to 95° C., preferably from 45 to 85° C.

Noble metal sensitizers for use in the noble metal sensitization include sensitizers of gold, platinum, palladium and iridium, and particularly, sensitizers of gold compounds are preferred. Examples of the gold sensitizers include chloroauric acid, potassium chloroaurate, potassium aurithiocyanate, gold sulfide and the like. They can be used in an amount of about  $1 \times 10^{-7}$  mol to about  $1 \times 10^{-2}$  mol based on one mole of silver halide.

Specific examples of the compound used in the reduction sensitization include an ascorbic acid, thiourea dioxide, stannous chloride, aminoiminomethanesulfonic acid, a hydrazine derivative, a borane compound, a silane compound and a polyamine compound. The reduction sensitization may be performed by ripening the grains while keeping the silver halide emulsion at a pH of 7 or more or at a pAg of 8.3 or less. The reduction sensitization may also be performed by introducing a single addition part of silver ion during the formation of grains.

The reducible silver salt used for the heat-developable photosensitive material of the present invention is relatively

stable against light, but forms a silver image when it is heated at 80° C. or higher in the presence of an exposed photocatalyst (e.g., a latent image of photosensitive silver halide) and a reducing agent. The organic silver salt may be any organic substance containing a source capable of reducing the silver ion. A silver salt of an organic acid, particularly a silver salt of a long chained aliphatic carboxylic acid (having from 10 to 30, preferably from 15 to 28 carbon atoms) is preferred. A complex of an organic or inorganic silver salt, whose ligand has a complex stability constant of from 4.0 to 10.0, is also preferred. The silver-supplying substance may constitute preferably from about 5 to 70% by weight of the image-forming layer. Examples of preferred organic silver salt include a silver salt of an organic compound having a carboxyl group. Examples include an aliphatic carboxylic acid silver salt and an aromatic carboxylic acid silver salt. However, the present invention is not limited to these examples. Preferred examples of the aliphatic carboxylic acid silver salt include silver behenate, silver arachidinate, silver stearate, silver oleate, silver laurate, silver caproate, silver myristate, silver palmitate, silver maleate, silver fumarate, silver tartrate, silver linoleate, silver butyrate, silver camphorate and a mixture thereof.

As the reducible silver salt, silver salts of compounds having mercapto or thione group and derivatives thereof may also be used as the organic silver salt. Preferred examples of these compounds include a silver salt of 3-mercaptop-4-phenyl-1,2,4-triazole, silver salt of 2-mercaptopbenzimidazole, silver salt of 2-mercaptop-5-aminothiadiazole, silver salt of 2-(ethylglycolamido) benzothiazole, silver salts of thioglycolic acids such as silver salts of S-alkylthioglycolic acids wherein the alkyl group has 12 to 22 carbon atoms, silver salts of dithiocarboxylic acids such as silver salt of dithioacetic acid, silver salts of thioamides, silver salt of 5-carboxyl-1-methyl-2-phenyl-4-thiopyridine, silver salts of mercaptotriazines, silver salt of 2-mercaptopbenzoxazole as well as silver salts of 1,2,4-mercaptopthiazole derivatives such as a silver salt of 3-amino-5-benzylthio-1,2,4-thiazole as described in U.S. Pat. No. 4,123,274 and silver salts of thione compounds such as silver salt of 3-(3-carboxyethyl)-4-methyl-4-thiazoline-2-thione as described in U.S. Pat. No. 3,301,678.

Compounds containing an imino group may also be used. Preferred examples of such a compound include silver salts of benzotriazole and derivatives thereof, for example, silver salts of benzotriazoles such as silver methylbenzotriazole, silver salts of halogenated benzotriazoles such as silver 5-chlorobenzotriazole as well as silver salts of 1,2,4-triazole and 1-H-tetrazole and silver salts of imidazole and imidazole derivatives as described in U.S. Pat. No. 4,220,709. Various silver acetylides compounds as described, for example, in U.S. Pat. Nos. 4,761,361 and 4,775,613 may also be used.

The reducible silver salt used for the present invention, i.e., the organic silver salt can be used for the present invention in a desired amount. For example, the organic silver salt may preferably be used in an amount of 0.1 to 5 g, more preferably 1 to 3 g per square meter of the heat-developable photosensitive material.

Although the shape of the organic silver salt is not particularly limited, an acicular crystal form having a short axis and a long axis is preferred. In the present invention, the short axis is preferably from 0.01 to 0.20  $\mu\text{m}$ , more preferably from 0.01 to 0.15  $\mu\text{m}$ , and the long axis is preferably from 0.10 to 5.0  $\mu\text{m}$ , more preferably from 0.10 to 4.0  $\mu\text{m}$ . The shape of the organic silver salt is determined from a transmission electron microscope image of organic silver salt dispersion.

The shape of the organic silver salt is not particularly limited. For example, however, its grain size determined by irradiating organic silver salt dispersed in a solution with a laser ray and determining an autocorrelation function of the fluctuation of the scattered light on the basis of the change in time (volume weight average diameter) is, in average, preferably from 0.05 to 10.0  $\mu\text{m}$ , more preferably from 0.1 to 5.0  $\mu\text{m}$ , further preferably from 0.1 to 2.0  $\mu\text{m}$ .

The grain size distribution of the organic silver salt is preferably monodisperse. The term "monodisperse" as used herein means that the percentage of the value obtained by dividing the standard deviation of the length of the short axis or long axis by the length of the short axis or long axis, respectively, is preferably 100% or less, more preferably 80% or less, and still more preferably 50% or less. Another method for determining the monodispersibility is a method involving obtaining the standard deviation of a volume weight average diameter of the organic silver salt. The percentage (coefficient of variation) of the value obtained by dividing the standard deviation by the volume weight average diameter is preferably 100% or less, more preferably 80% or less, still more preferably 50% or less.

The organic silver salt used in the present invention is preferably desalinated. The desalting method is not particularly limited and any known method may be used. Known filtration methods such as centrifugal filtration, suction filtration, ultrafiltration and flocculation washing by coagulation may be preferably used.

In the present invention, for obtaining an organic silver salt solid dispersion having a high SIN ratio and a small grain size and being free from coagulation, preferably used is a dispersion method comprising the steps of converting a water dispersion, that contains an organic silver salt as an image-forming medium, to a high-speed flow dispersion, and then releasing the pressure. That is, the method comprises steps of supplying a water dispersion containing at least an organic silver salt under a positive pressure by means of a high-pressure pump or the like into a pipeline, passing the dispersion through a narrow slit provided inside the pipeline, and then subjecting the dispersion to rapid pressure reduction to perform fine dispersion.

The above-described water dispersion obtained using conversion under a high-pressure and at high-speed flow is substantially free of a photosensitive silver salt. The content thereof is 0.1 mol % or less based on the light-insensitive organic silver salt. A photosensitive silver salt may not be added intentionally.

The solid dispersing apparatus and technique used for performing the above-described dispersion method in the present invention are described in detail, for example, in Toshio Kajuchi and Hiromoto Usui, Bunsan-Kei Rheology to Bunsanka Gijutsu (Rheology of Dispersion System and Dispersion Technology), pp.357-403, Shinzan Sha Shuppan (1991), and Kagaku Kogaku no Shinpo (Progress of Chemical Engineering), pp. 184-185, compiled by Corporation Kagaku Kogakukai Tokai Shibu, Maki Shoten (1990).

As for the high-pressure homogenizer which may be used in the present invention, it is considered that the dispersion into fine grains is generally achieved by dispersion forces such as (a) "shear force" generated at the passage of a dispersoid through a narrow slit under a high pressure at a high speed, and (b) "cavitation force" generated at the time of the release of the dispersoid from the high pressure so as to be under normal pressure. As the dispersion apparatus of this class, an example include the Golline homogenizer previously used. By using this apparatus, the solution to be dispersed is transported under a high pressure and converted

into a high-speed flow through a narrow slit on the cylinder surface, and the energy of the flow allows collision of the flow against the peripheral wall surface to achieve emulsification and dispersion. The pressure applied may generally be from 100 to 600 kg/cm<sup>2</sup> and the flow velocity may be from several m/sec to 30 m/sec. In order to increase the dispersion efficiency, some apparatuses are designed wherein a part of a high flow velocity is formed into a serrated shape to increase the frequency of collision. Apparatuses capable of dispersion under a higher pressure and at a higher flow velocity have been developed in recent years, and examples include Microfluidizer (manufactured by Microfluidex International Corporation) and Nanomizer (manufactured by Tokusho Kika Kogyo KK).

Examples of the dispersing apparatus which can be suitably used in the present invention include Microfluidizer M-110S-EH (with G10Z interaction chamber), M-110Y (with H10Z interaction chamber), M-140K (with G10Z interaction chamber), HC-5000 (with L30Z or H230Z interaction chamber) and HC-8000 (with E230Z or L30Z interaction chamber), all manufactured by Microfluidex International Corporation.

By using these apparatuses, an aqueous dispersion containing at least an organic silver salt is transported under a positive pressure by means of a high-pressure pump or the like into the pipeline, and the solution is passed though a narrow slit provided inside the pipeline to apply a desired pressure. Then, the pressure in the pipeline is rapidly released to the atmospheric pressure to apply a rapid pressure change to the dispersion to obtain an optimal organic silver salt dispersion for use in the present invention.

In dispersing process of the organic silver salt for use in the present invention, dispersion having a desired grain size may be obtained by controlling the flow velocity, the difference in the pressure before and after at the pressure dropping and the frequency of the processing. From viewpoints of photographic performance and the grain size, the flow velocity is preferably from 200 to 600 m/sec and the difference in the pressure at the pressure dropping is preferably from 900 to 3,000 kg/cm<sup>2</sup>, and more preferably, the flow velocity is from 300 to 600 m/sec, and the difference in the pressure at the pressure dropping is from 1,500 to 3,000 kg/cm<sup>2</sup>. The frequency of the dispersion processing may be appropriately chosen as required, and is usually from 1 to 10 times. From a viewpoint of productivity, the frequency is approximately from 1 to 3 times. The water dispersion under a high pressure is preferably not warmed at a high temperature from viewpoints of dispersibility and photographic performance. At a high temperature above 90° C., a grain size may readily become large and fog may be increased. Accordingly, in the present invention, the water dispersion is preferably kept at a temperature of from 5 to 90° C., more preferably from 5 to 80° C., and most preferably from 5 to 65° C., by providing a cooling step before the conversion into a high pressure and high flow velocity, after the pressure drop, or both before the conversion and after the pressure drop. It is particularly effective to provide the cooling step at the time of dispersion under a high pressure of from 1,500 to 3,000 kg/cm<sup>2</sup>. The cooler may be appropriately selected from a double pipe, a double piper using a static mixer, a multi-tubular exchanger and a coiled heat exchanger, depending on an amount of heat exchange to be treated. The size, wall thickness or material of a pipe may be appropriately selected to increase heat exchange efficiency depending on an applied pressure. In addition, depending on an amount of heat exchange, a refrigerant used in the cooler may be a well water at 20° C. or a chilled water at from 5

45

to 10° C. cooled by a refrigerator, and if desired, a refrigerant such as ethylene glycol/water at 30° C. may also be used.

In the dispersion operation, the organic silver salt is preferably dispersed in the presence of a dispersant (dispersion aid) soluble in an aqueous solvent. Examples of the dispersion aid include synthetic anion polymers such as polyacrylic acid, copolymer of acrylic acid, maleic acid copolymer, maleic acid monoester copolymer and acrylomethylpropanesulfonic acid copolymer, semisynthetic anion polymers such as carboxymethyl starch and carboxymethyl cellulose, anionic polymers such as alginic acid and pectic acid, compounds described in JP-A-7-350753, known anionic, nonionic or cationic surface active agents, known polymers such as polyvinyl alcohol, polyvinyl pyrrolidone, carboxymethyl cellulose, hydroxypropyl cellulose and hydroxypropylmethyl cellulose, and naturally-occurring polymer compounds such as gelatin, and these may be appropriately selected and used. Polyvinyl alcohols and water-soluble cellulose derivatives are particularly preferred.

The dispersing aid is generally mixed with the organic silver salt in a form of powder or wet cake before the dispersing process, and fed as slurry into a dispersing apparatus. The dispersing aid may be mixed with the organic silver salt beforehand, and then the mixture may be subjected to a treatment such as by heating or with a solvent to form an organic silver salt powder or wet cake. The pH may be controlled with a suitable pH modifier before, during or after the dispersing operation.

Other than the mechanical dispersion, the organic silver salt can be made into fine grains by roughly dispersing the salt in a solvent through pH control, and then changing the pH in the presence of a dispersant. For the operation, an organic solvent may be used as a solvent for the rough dispersion, and such organic solvent can be removed after the formation of grains.

The prepared dispersion of the organic silver salt can be stored with stirring to prevent precipitation of the grains during storage, or stored in a highly viscous state by means of a hydrophilic colloids (e.g., a jelly state formed with gelatin). Furthermore, the dispersion may contain a preservative in order to prevent proliferation of microorganisms during storage.

The dispersion of the organic silver salt thus obtained is then mixed with an aqueous photosensitive silver salt solution to produce a coating solution containing the photosensitive image-forming medium. The coating solution enables the manufacture of a heat-developable photosensitive material exhibiting low haze and low fog, and having high sensitivity. When a photosensitive silver salt coexists at the time of dispersing process under a high-pressure and at high-speed flow, fog frequency may increase and sensitivity may often highly decrease. Furthermore, when an organic solvent is used as a dispersion medium instead of water, haze and fog may increase and sensitivity may likely be decreased. When a conversion method where a part of the organic silver salt in the dispersion is converted into a photosensitive silver salt is used instead of the method of mixing an aqueous photosensitive silver salt solution, sensitivity may likely be decreased.

Examples of a method and conditions for mixing the photosensitive silver halide with a separately prepared organic silver salt include, for example, a method of mixing the silver halide grains and the organic silver salt by means of a high-speed stirrer, a ball mill, a sand mill, a colloidal mill, a vibration mill, a homogenizer or the like, or a method

46

of adding a ready prepared photosensitive silver halide to an organic silver salt at any stage of its preparation. However, the mixing method and conditions are not particularly limited so long as the advantages of the invention can be fully achieved.

The heat-developable photosensitive material of the present invention comprises a binder on the same side of a support as that provided with the aforementioned photosensitive silver halide and the reducible silver salt. The binder of the image-forming layer (photosensitive layer, emulsion layer) can be selected from well known natural or synthetic resins such as gelatin, poly(vinyl acetal), poly(vinyl chloride), poly(vinyl acetate), cellulose acetate, polyolefins, polyesters, polystyrene, polyacrylonitrile and polycarbonates. Copolymers and terpolymers may also be used, of course. Preferred polymers are polyvinyl butyral, butyl ethyl cellulose, methacrylate copolymer, maleic anhydride ester copolymer, polystyrene and butadiene/styrene copolymer. Two or more of these polymers can be used in combination, if required. The polymers are used in an amount sufficient to hold other components in the polymer, namely, they are used in an effective range to function as a binder. Those skilled in the art can appropriately determine the effective range. In order to hold at least the organic silver salt, a guide of the proportion of the binder to the organic silver salt may preferably range from 15:1 to 1:2, more preferably from 8:1 to 1:1.

At least one of layers constituting the image-forming layer is preferably an image-forming layer containing at least 50% by weight of polymer latex described below based on the total binder thereof (hereinafter in the specification, such an image-forming layer is referred to as the "image-forming layer of the present invention", and the polymer latex used for the binder is referred to as the "polymer latex of the present invention"). The polymer latex may be used not only in the image-forming layer, but in a protective layer and a backing layer. When the heat-developable photosensitive material of the present invention is used for printing in which a dimensional change causes a problem, the polymer latex needs to be used also in the protective layer and the backing layer. The term "polymer latex" used herein means a material comprising water-insoluble hydrophobic polymer fine particles dispersed in a water-soluble dispersion medium. As for a dispersion state, the polymers may be those emulsified in a dispersion medium, those obtained by an emulsion-polymerization, or those obtained by a micell dispersion, or those having a partially hydrophilic structure in their molecule so as to allow molecular dispersion of the molecular chain. The polymer latex for use in the present invention is described in Gosei Jushi Emulsion (Synthetic Resin Emulsion), compiled by Taira Okuda and Hiroshi Inagaki, issued by Kobunshi Kanko Kai (1978), Gosei Latex no Oyo (Application of Synthetic Latex), compiled by Takaaki Sugimura, Yasuo Kataoka, Souichi Suzuki and Keiji Kasahara, issued by Kobunshi Kanko Kai (1993), and Soichi Muroi, Gosei Latex no Kagaku (Chemistry of Synthetic Latex), Kobunshi Kanko Kai (1970) and the like. The dispersion particles preferably have an average particle size of from 1 to 50,000 nm, more preferably from 5 to 1,000 nm. The particle size distribution of the dispersed particles is not particularly limited, and the dispersed particles may have a broad particle size distribution or a monodisperse particle size distribution.

As the polymer latex used for the present invention, a so-called core/shell type latex may be used, as well as the normal polymer latex having a uniform structure. Where the core/shell latex is used, preferable properties may some-

times be obtained when a core and a shell have different glass transition temperatures.

The polymer latexes used as the binders for a protective layer, a backing layer, and an image-forming layer have different respective preferred ranges of glass transition temperature (Tg). For the image-forming layer, the glass transition temperature is preferably 40° C. or lower, more preferably from 30° C. to 40° C. to accelerate the diffusion of the photographically useful materials during the heat development. For the protective layer and the backing layer, the glass transition temperature is preferably 25° C. to 70° C. to protect from damages by contact with various instruments.

The polymer latex for use in the present invention preferably has a minimum film-forming temperature (MFT) of from 30 to 90° C., more preferably from 0 to 70° C. In order to control the minimum film-forming temperature, a film-forming aid may be added. The film-forming aid is also called a plasticizer and is an organic compound (usually an organic solvent) capable of decreasing the minimum film-forming temperature of the polymer latex. Such organic compounds are described in, for example, Souichi Muroi, Gosei Latex no Kagaku (Chemistry of Synthetic Latex), Kobunshi Kankō Kai (1970) mentioned above.

Examples of the polymer used as the polymer latex include acrylic resin, vinyl acetate resin, polyester resin, polyurethane resin, rubber-based resin, vinyl chloride resin, vinylidene chloride resin, polyolefin resin or a copolymer thereof. The polymer may be a straight-chained polymer, a branched polymer or a cross-linked polymer. The polymer may also be a so-called homopolymer obtained by polymerizing a single monomer or may be a copolymer obtained by polymerizing two or more of monomers. The copolymer may be either a random copolymer or a block copolymer. The polymer has a number average molecular weight of from 5,000 to 1,000,000, preferably from 10,000 to 100,000. If the molecular weight is too small, the image-forming layer may sometimes be deficient in mechanical strength, whereas if the molecular weight is too large, the film-forming property may sometimes be poor.

Examples of the polymer latex used as the binder in the image-forming layer of the heat-developable image-recording material of the present invention include, for example, a methyl methacrylate/ethyl acrylate/methacrylic acid copolymer latex, methyl methacrylate/2-ethylhexyl acrylate/styrene/acrylic acid copolymer latex, styrene/butadiene/acrylic acid copolymer latex, styrene/butadiene/divinylbenzene/methacrylic acid copolymer latex, methyl methacrylate/vinyl chloride/acrylic acid copolymer latex, vinylidene chloride/ethyl acrylate/acrylonitrile/methacrylic acid copolymer latex and the like. Such polymers are commercially available and the following polymers can be used: acrylic resins such as CEBIAN A-4635, 46583, 4601 (all produced by Dicel Kagaku Kogyo Co., Ltd), Nipol Lx811, 814, 821, 820, and 857 (all produced by Nippon Zeon Co., Ltd.); polyester resins such as FINETEX ES650, 611, 675, 850 (all produced by Dai-Nippon Ink & Chemicals, Inc.), WD-size and WMS (both produced by Eastman Chemical); polyurethane resins such as HYDRAN AP10, 20, 30, and 40 (all produced by Dai-Nippon Ink & Chemicals, Inc.); rubber-based resins such as LACSTAR 7310K, 3307B, 4700H, 7132C, (all produced by Dai-Nippon Ink & Chemicals, Inc.), Nipol Lx416, 410, 438C, and 2507 (all produced by Nippon Zeon Co., Ltd.); vinyl chloride resins such as G351, and G576 (both produced by Nippon Zeon Co., Ltd.); vinylidene chloride resins such as L502, L513 (both produced by Asahi Chemical Industry

Co., Ltd.), ARON D7020, D504, and D5071 (all produced by Toagosei Co., Ltd.); and olefin resins such as CHEMIPEARL S120 and SA100 (both produced by Mitsui Petrochemical Industries, Ltd.) and the like. These polymers may be used alone or as a blend of two or more of the polymers, if desired.

The image-forming layer of the heat-developable photosensitive layer according to the present invention preferably contains 50% by weight or more, more preferably 70% by weight or more of the aforementioned polymer latex based on the total binder.

If desired, the image-forming layer of the heat-developable photosensitive layer according to the present invention may contain a hydrophilic polymer in an amount of 50% by weight or less of the total binder, such as gelatin, polyvinyl alcohol, methyl cellulose, hydroxypropyl cellulose, carboxymethyl cellulose and hydroxypropylmethyl cellulose. The amount of the hydrophilic polymer added is preferably 30% by weight or less, more preferably 15% by weight of the total binder in the image-forming layer.

The image-forming layer of the present invention is preferably formed by coating an aqueous coating solution and then drying the coating solution. The term "aqueous" as used herein means that water content of the solvent (dispersion medium) in the coating solution is 60% by weight or more. In the coating solution, the component other than water may be a water-miscible organic solvent such as methyl alcohol, ethyl alcohol, isopropyl alcohol, methyl cellosolve, ethyl cellosolve, dimethylformamide, and ethyl acetate. Examples of the solvent composition include water/methanol=90/10, water/methanol=70/30, water/ethanol=90/10, water/isopropanol=90/10, water/dimethylformamide=95/5, water/methanol/dimethylformamide=80/15/5 and water/methanol/dimethylformamide=90/5/5 (the numerals are in % by weight) as well as water alone.

The total amount of the binder in the image-forming layer according to the present invention is preferably from 0.2 to 30 g/m<sup>2</sup>, more preferably from 1 to 15 g/m<sup>2</sup>. The image-forming layer of the present invention may contain a crosslinking agent for cross-linkage, a surfactant for improving coating property and the like.

The heat-developable photosensitive material of the present invention preferably contains an ultrahigh contrast agent. As the ultrahigh contrast agent, preferred are one or more of a substituted alkene derivative represented by the following formula (17), a substituted isoxazole derivative represented by the following formula (18), and a compound represented by the following formula (19).



-continued



(19)

In the formula (17),  $R^{1a}$ ,  $R^{2a}$  and  $R^{3a}$  each independently represents a hydrogen atom or a functional group, and  $Z$  represents an electron withdrawing group or a silyl group.  $R^{1a}$  together with  $Z$ ,  $R^{2a}$  together with  $R^{3a}$ ,  $R^{1a}$  together with  $R^{2a}$ , or  $R^{3a}$  together with  $Z$  may combine with each other to form a ring structure. In the formula (18),  $R^{4a}$  represents a functional group; and in the formula (19),  $X$  and  $Y$  independently represent a hydrogen atom or a functional group,  $A$  and  $B$  independently represent an alkoxy group, an alkylthio group, an alkylamino group, an aryloxy group, an arylthio group, an anilino group, a heterocyclyloxy group, a heterocyclythio group or a heterocyclamino group, and  $X$  together with  $Y$ , or  $A$  together with  $B$  may be combined with each other to form a ring structure.

The substituted alkene derivatives represented by the formula (17) will be explained in detail below.

In the formula (17),  $R^{1a}$ ,  $R^{2a}$  and  $R^{3a}$  independently represent a hydrogen atom or a functional group, and  $Z$  represents an electron withdrawing group or a silyl group. In the formula (17),  $R^{1a}$  together with  $Z$ ,  $R^{2a}$  together with  $R^{3a}$ ,  $R^{1a}$  together with  $R^{2a}$ , or  $R^{3a}$  together with  $Z$  may combine with each other to form a ring structure.

When  $R^{1a}$ ,  $R^{2a}$  or  $R^{3a}$  represents a functional group, examples of the functional group include a halogen atom (e.g., fluorine, chlorine, bromide, iodine), an alkyl group (including an aralkyl group, a cycloalkyl group and active methine group), an alkenyl group, an alkynyl group, an aryl group, a heterocyclic group (including N-substituted nitrogen-containing heterocyclic group), a quaternized nitrogen-containing heterocyclic group (e.g., pyridinio group), an acyl group, an alkoxy carbonyl group, an aryloxy carbonyl group, a carbamoyl group, carboxyl group or a salt thereof, an imino group, an imino group substituted at N atom, a thiocarbonyl group, a sulfonyl carbamoyl group, an acyl carbamoyl group, a sulfamoyl carbamoyl group, a carbazoyl group, an oxazyl group, an oxamoyl group, cyano group, a thiocarbamoyl group, hydroxyl group (or a salt thereof), an alkoxy group (including a group containing ethyleneoxy group or propyleneoxy group repeating unit), an aryloxy group, a heterocyclyloxy group, an acyloxy group, an (alkoxyl or aryloxy) carbonyloxy group, a carbamoyloxy group, a sulfonyloxy group, an amino group, an (alkyl, aryl or heterocyclic)amino group, an acylamino group, a sulfonamido group, a ureido group, a thioureido group, an imido group, an (alkoxyl or aryloxy) carbonylamino group, a sulfamoylamino group, a semicarbazide group, a thiosemicarbazide group, a hydrazino group, a quaternary ammonio group, an oxamoylamino group, an (alkyl or aryl)sulfonylureido group, an acylureido group, an acylsulfamoylamino group, nitro group, mercapto group, an (alkyl, aryl or heterocyclic)thio group, an acylthio group, an (alkyl or aryl)sulfonyl group, an (alkyl or aryl)sulfinyl group, sulfo group or a salt thereof, a sulfamoyl group, an acylsulfamoyl group, a sulfonylsulfamoyl group or a salt thereof, a phosphoryl group, a group containing phosphoramido or phosphoric acid ester structure, a silyl group and a stannyl group. These functional groups may further be substituted with any one or more of the above-described functional groups.

The electron withdrawing group represented by  $Z$  is a functional group that gives a positive value of the Ham-

mett's functional group constant  $\sigma_p$ , and specific examples include those exemplified for  $R^1$  and  $R^2$  in the general formula (2). The electron withdrawing group represented by  $Z$  may further have one or more functional groups, and 5 examples of the functional groups include those described as the functional group represented by  $R^{1a}$ ,  $R^{2a}$  or  $R^{3a}$  in the formula (17).

$R^{1a}$  together with  $Z$ ,  $R^{2a}$  together with  $R^{3a}$ ,  $R^{1a}$  together with  $R^{2a}$ , or  $R^{3a}$  together with  $Z$  may combine with each 10 other to form a ring structure. The ring structure formed is a non-aromatic carbocyclic ring or a non-aromatic heterocyclic ring.

The preferred scope of the substituted alkene derivatives represented by the formula (17) will be described below.

15 The functional group represented by  $R^{1a}$ ,  $R^{2a}$  or  $R^{3a}$  in the formula (17) may preferably be a group having a total carbon atom number of from 0 to 30, and specific examples of the group include the same groups as those explained as the electron withdrawing group represented by  $Z$  in the formula (17), as well as an alkyl group, hydroxyl group (or a salt thereof), mercapto group (or a salt thereof), an alkoxy group, an aryloxy group, a heterocyclyloxy group, an alkylthio group, an arylthio group, a heterocyclythio group, an amino group, an alkylamino group, an arylamino group, a heterocyclamino group, a ureido group, an acylamino group, 25 a sulfonamido group and a substituted, unsubstituted aryl group and the like.

20  $R^{1a}$  is preferably an electron withdrawing group, an aryl group, an alkylthio group, an alkoxy group, an acylamino group, hydrogen atom, or a silyl group.

When  $R^{1a}$  represents an electron withdrawing group, the 25 electron withdrawing group may preferably be a group having a total carbon atom number of from 0 to 30 such as cyano group, nitro group, an acyl group, a formyl group, an alkoxy carbonyl group, an aryloxycarbonyl group, a thiocarbonyl group, an imino group, an imino group substituted at N atom, an alkylsulfonyl group, an arylsulfonyl group, a carbamoyl group, a sulfamoyl group, a trifluoromethyl group, a phosphoryl group, carboxyl group (or a salt thereof), a saturated or unsaturated heterocyclic group, more 30 preferably cyano group, an acyl group, a formyl group, an alkoxy carbonyl group, a carbamoyl group, an imino group, an imino group substituted at N atom, a sulfamoyl group, carboxyl group (or a salt thereof) or a saturated or unsaturated heterocyclic group, and most preferably cyano group, a formyl group, an acyl group, an alkoxy carbonyl group, a carbamoyl group or a saturated or unsaturated heterocyclic group.

35 When  $R^{1a}$  represents an aryl group, the aryl group is 40 preferably a substituted or unsubstituted phenyl group having a total carbon atom number of from 6 to 30. The functional group may be any functional group, and an electron withdrawing functional group is preferred. 45  $R^{1a}$  is more preferably an electron withdrawing group or an aryl group.

The functional group represented by  $R^{2a}$  or  $R^{3a}$  may 50 preferably be the same group as those explained as the electron withdrawing group represented by  $Z$  in the formula (17), as well as an alkyl group, hydroxyl group (or a salt thereof), mercapto group (or a salt thereof), an alkoxy group, an aryloxy group, a heterocyclyloxy group, an alkylthio group, an arylthio group, a heterocyclythio group, an amino group, an alkylamino group, an arylamino group, a heterocyclamino group, an acylamino group or a substituted 55 or unsubstituted phenyl group.

It is more preferred that one of  $R^{2a}$  and  $R^{3a}$  is hydrogen atom and the other is a functional group. The functional

group may preferably be an alkyl group, hydroxyl group (or a salt thereof), mercapto group (or a salt thereof), an alkoxy group, an aryloxy group, a heterocyclyloxy group, an alkylthio group, an arylthio group, a heterocyclylthio group, an amino group, an alkylamino group, an anilino group, a heterocyclamino group, an acylamino group (particularly, a perfluoroalkanamido group), a sulfonamido group, a substituted or unsubstituted phenyl group or a heterocyclic group, more preferably hydroxyl group (or a salt thereof), mercapto group (or a salt thereof), an alkoxy group, an aryloxy group, a heterocyclyloxy group, an alkylthio group, an arylthio group, a heterocyclylthio group or a heterocyclic group, and most preferably hydroxyl group (or a salt thereof), an alkoxy group or a heterocyclic group.

When Z represents a silyl group, it may preferably be trimethylsilyl group, t-butyldimethylsilyl group, phenyldimethylsilyl group, triethylsilyl group, triisopropylsilyl group or trimethylsilyldimethylsilyl group.

When Z represents an electron withdrawing group, it may preferably be a group having a total carbon atom number of from 0 to 30 such as, specifically, cyano group, an alkoxy-carbonyl group, an aryloxycarbonyl group, a carbamoyl group, a thiocarbonyl group, an imino group, an imino group substituted at N atom, a sulfamoyl group, an alkylsulfonyl group, an arylsulfonyl group, nitro group, a perfluoroalkyl group, an acyl group, a formyl group, a phosphoryl group, an acyloxy group, an acylthio group or a phenyl group substituted with one or more electron withdrawing groups, more preferably cyano group, an alkoxy-carbonyl group, a carbamoyl group, an imino group, a sulfamoyl group, an alkylsulfonyl group, an arylsulfonyl group, an acyl group, a formyl group, a phosphoryl group, a trifluoromethyl group, or a phenyl group substituted with one or more electron withdrawing group, and most preferably cyano group, a formyl group, an acyl group, an alkoxy-carbonyl group, an imino group or a carbamoyl group.

Z is more preferably an electron withdrawing group.

It is also preferred that Z together with R<sup>1a</sup> or R<sup>2a</sup> together with R<sup>3a</sup> form a ring structure. As the ring structure, a 5-, 6- or 7-membered ring is preferred, more preferably such a ring having a total carbon atom number, including those of functional groups thereon, of from 1 to 40, further preferably from 3 to 30.

The substituted alkene derivative represented by the formula (17) is more preferably a compound wherein R<sup>1a</sup> represents an electron withdrawing group or an aryl group, one of R<sup>2a</sup> and R<sup>3a</sup> represents hydrogen atom and the other represents hydroxyl group (or a salt thereof), mercapto group (or a salt thereof), an alkoxy group, an aryloxy group, a heterocyclyloxy group, an alkylthio group, an arylthio group, a heterocyclylthio group or a heterocyclic group, and Z represents cyano group, a formyl group, an acyl group, an alkoxy-carbonyl group, an imino group or a carbamoyl group; and a compound wherein R<sup>1a</sup> and Z form a non-aromatic 5-, 6- or 7-membered ring structure, and one of R<sup>2a</sup> and R<sup>3a</sup> represents hydrogen atom and the other represents hydroxyl group (or a salt thereof), mercapto group (or a salt thereof), an alkoxy group, an aryloxy group, a heterocyclyloxy group, an alkylthio group, an arylthio group, a heterocyclylthio group or a heterocyclic group. In the latter compound, Z which forms a non-aromatic ring structure together with R<sup>1a</sup> is preferably an acyl group, a carbamoyl group, an oxycarbonyl group, a thiocarbonyl group or a sulfonyl group (a hydrogen atom contained in these group is replaced with a part of R<sup>1a</sup>), and R<sup>1a</sup> is preferably an acyl group, a carbamoyl group, an oxycarbonyl group, a thiocarbonyl group, a sulfonyl group, an imino group, an imino

group substituted at N atom, an acylamino group or a carbonylthio group (a hydrogen atom contained in these group is replaced with a part of Z).

The substituted isoxazole derivative represented by the formula (18) will be described in detail below.

In the formula (18), examples of the functional group represented by R<sup>4a</sup> include those explained as the functional group represented by R<sup>1a</sup>, R<sup>2a</sup> or R<sup>3a</sup> in the formula (17). The functional group represented by R<sup>4</sup> may preferably be an electron withdrawing group or an aryl group.

Where R<sup>4a</sup> represents an electron withdrawing group, the electron withdrawing group may preferably be a group having a total carbon atom number of from 0 to 30 such as, specifically, cyano group, nitro group, an acyl group, a formyl group, an alkoxy-carbonyl group, an aryloxycarbonyl group, an alkylsulfonyl group, an arylsulfonyl group, a carbamoyl group, a sulfamoyl group, a trifluoromethyl group, a phosphoryl group, an imino group or a saturated or unsaturated heterocyclic group, more preferably cyano group, an acyl group, a formyl group, an alkoxy-carbonyl group, a carbamoyl group, a sulfamoyl group, an arylsulfonyl group, a carbamoyl group, a sulfamoyl group, an alkylsulfonyl group, an arylsulfonyl group or a heterocyclic group, and most preferably cyano group, a formyl group, an acyl group, an alkoxy-carbonyl group, a carbamoyl group or a heterocyclic group.

Where R<sup>4a</sup> represents an aryl group, the aryl group may preferably be a substituted or unsubstituted phenyl group having a total carbon atom number of from 0 to 30. Examples of the functional group include those described as the functional group represented by R<sup>1a</sup>, R<sup>2a</sup> or R<sup>3a</sup> in the formula (17).

R<sup>4a</sup> is more preferably cyano group, an alkoxy-carbonyl group, a carbamoyl group, a heterocyclic group or a substituted or unsubstituted phenyl group, and most preferably cyano group, a heterocyclic group or an alkoxy-carbonyl group.

The compound represented by the formula (19) will be described in detail below.

In the formula (19), X and Y independently represent hydrogen atom or a functional group, and A and B independently represent an alkoxy group, an alkylthio group, an alkylamino group, an aryloxy group, an arylthio group, an anilino group, a heterocyclyloxy group, a heterocyclylthio group or a heterocyclamino group, and X together with Y or A together with B may combine with each other to form a ring structure.

Examples of the functional group represented by X or Y in the formula (19) include those described as the functional group represented by R<sup>1a</sup>, R<sup>2a</sup> or R<sup>3a</sup> in the formula (17). These groups may further have one or more functional groups. X together with Y may combine with each other to form a ring structure, and the ring structure formed may be either a non-aromatic carbocyclic ring or a non-aromatic heterocyclic ring.

Where X and Y represent functional groups, they may preferably be a functional group having a total carbon number of from 1 to 40, more preferably from 1 to 30, such as, specifically, cyano group, an alkoxy-carbonyl group, an aryloxycarbonyl group, a carbamoyl group, an imino group, an imino group substituted at the nitrogen atom, a thiocarbonyl group, a sulfamoyl group, an alkylsulfonyl group, an arylsulfonyl group, nitro group, a perfluoroalkyl group, an acyl group, a formyl group, a phosphoryl group, an acylamino group, an acyloxy group, an acylthio group, a heterocyclic group, an alkylthio group, an alkoxy group or an aryl group.

X and Y are more preferably cyano group, nitro group, an alkoxy-carbonyl group, a carbamoyl group, an acyl group, a

formyl group, an acylthio group, an acylamino group, a thiocarbonyl group, a sulfamoyl group, an alkylsulfonyl group, an arylsulfonyl group, an imino group, an imino group substituted at the nitrogen atom, a phosphoryl group, a trifluoromethyl group, a heterocyclic group, a substituted phenyl group or the like, further preferably cyano group, an alkoxy carbonyl group, a carbamoyl group, an alkylsulfonyl group, an arylsulfonyl group, an acyl group, an acylthio group, an acylamino group, a thiocarbonyl group, a formyl group, an amino group, an imino group substituted at N atom, a heterocyclic group a phenyl group substituted by any electron withdrawing group or the like.

X and Y may also preferably combine with each other to form a ring structure. The ring structure is preferably a 5-, 6- or 7-membered ring, more preferably such a ring having a total carbon atom number of from 1 to 40, further preferably from 3 to 30. X and Y for forming a ring structure are preferably an acyl group, a carbamoyl group, an oxy carbonyl group, a thiocarbonyl group, a sulfonyl group, an imino group, an imino group substituted at the nitrogen atom, an acylamino group, a carbonylthio group (a hydrogen atom contained in these group is replaced with a part of X or Y) or the like.

A and B independently represent an alkoxy group, an alkylthio group, an alkylamino group, an aryloxy group, an arylthio group, an anilino group, a heterocyclyloxy group, a heterocyclylthio group or a heterocyclylamino group, which may combine with each other to form a ring structure.

The functional groups represented by A and B are preferably a group having a total carbon atom number of from 1 to 40, more preferably from 1 to 30, and the group may further have one or more functional groups.

A and B more preferably combine with each other to form a ring structure. The ring structure formed is preferably a 5-, 6- or 7-membered non-aromatic heterocyclic ring having a total carbon atom number of from 1 to 40, more preferably from 3 to 30. Examples of a structure (—A—B—) formed by the linking of A and B include —O—(CH<sub>2</sub>)<sub>2</sub>—O—, —O—(CH<sub>2</sub>)<sub>3</sub>—O—, —S—(CH<sub>2</sub>)<sub>2</sub>—S—, —S—(CH<sub>2</sub>)<sub>3</sub>—S—, —S—ph-S—, —N(CH<sub>3</sub>)—(CH<sub>2</sub>)<sub>2</sub>—O—, —N(CH<sub>3</sub>)—(CH<sub>2</sub>)<sub>2</sub>—S—, —O—(CH<sub>2</sub>)<sub>2</sub>—S—, —O—(CH<sub>2</sub>)<sub>3</sub>—S—, —N(CH<sub>3</sub>)—ph-O—, —N(CH<sub>3</sub>)—ph-S—, —N(ph)—(CH<sub>2</sub>)<sub>2</sub>—S— and the like.

The ultrahigh contrast agent compound represented by the formula (17), (18) or (19) preferably used in the present invention may be introduced with a group capable of adsorb-

ing to silver halide. Examples of the adsorbing group include the groups described in U.S. Pat. Nos. 4,385,108 and 4,459,347, JP-A-59-195233, JP-A-59-200231, JP-A-59-201045, JP-A-59-201046, JP-A-59-201047, JP-A-59-201048, JP-A-59-201049, JP-A-61-170733, JP-A-61-270744, JP-A-62-948, JP-A-63-234244, JP-A-63-234245 and JP-A-63-234246, such as an alkylthio group, an arylthio group, a thiourea group, a thioamide group, a mercaptoheterocyclic group and a triazole group. The adsorbing group to silver halide may be formed as a precursor. Examples of the precursor include the groups described in JP-A-2-285344.

The compound represented by the formula (17), (18) or (19) may be introduced with a ballast group or a polymer commonly used in the field of immobile photographic additives such as a coupler. The compounds incorporated with the ballast group may be preferred for the present invention. The ballast group is a group having 8 or more carbon atoms and being relatively inactive in the photographic performance. Examples of the ballast group include an alkyl group, an aralkyl group, an alkoxyl group, a phenyl group, an alkylphenyl group, a phenoxy group, an alkylphenoxy group and the like. Examples of the polymer include those described in JP-A-1-100530 and the like.

The compound represented by the formula (17), (18) or (19) may contain a cationic group (specifically, a group containing a quaternary ammonium group or a nitrogen-containing heterocyclic group containing a quaternized nitrogen atom), a group containing an ethyleneoxy group or a propyleneoxy group as a repeating unit, an (alkyl, aryl or heterocyclic)thio group, or a dissociative group capable of dissociation by a base (e.g., carboxyl group, sulfo group, an acylsulfamoyl group, a carbamoylsulfamoyl group), preferably a group containing an ethyleneoxy group or a propyleneoxy group as a repeating unit, or an (alkyl, aryl or heterocyclic)thio group. Specific examples of these groups include the compounds described in JP-A-7-234471, JP-A-5-333466, JP-A-6-19032, JP-A-6-19031, JP-A-5-45761, U.S. Pat. Nos. 4,994,365 and 4,988,604, JP-A-3-259240, JP-A-7-5610, JP-A-7-244348 and German Patent No. 4,006,032.

Specific examples of the ultrahigh contrast agent compounds represented by the formulae (17) to (19) preferably used in the present invention are shown below. However, the ultrahigh contrast agent used in the present invention is not limited to the following compounds.





-continued

B-7



B-8



B-9



B-10



B-11



B-12



B-13



B-14



B-15



B-16



B-17



B-18



B-19



B-20



B-21



B-22

-continued



B-23



B-25



B-27



B-29



B-31



B-33



B-35



B-24

B-26

B-28

B-30

B-32

B-34

B-36

**59****60**

-continued

B-37



B-38

B-39



B-40

B-41



B-42

B-43



B-44

B-45



B-46

**61****62**

-continued

B-47



B-48



B-49



B-50



B-51

B-52



B-53

B-54



B-55

B-56



-continued

B-57

B-58



B-59



B-60



The ultrahigh contrast agent compounds represented by formulae (17) to (19) can be easily synthesized according to known methods. For example, the compounds and may be synthesized by referring to the methods described in U.S. Pat. Nos. 5,545,515, 5,635,339 and 5,654,130, International Patent Publication WO97/34196 or Japanese Patent Application Nos. 9-354107, 9-309813 and 9-272002.

The amount of the ultrahigh contrast agent preferably used in the present invention is preferably from  $1 \times 10^{-6}$  to 1 mol, more preferably from  $1 \times 10^{-5}$  to  $5 \times 10^{-1}$  mol, most preferably from  $2 \times 10^{-5}$  to  $2 \times 10^{-1}$  mol based on per mole of silver.

The ultrahigh contrast agent may be used alone or in combination of two or more compounds. In addition to the compounds represented by the formulae (17) to (19), any of the compounds described in U.S. Pat. Nos. 5,545,515, 5,635,339 and 5,654,130, International Patent Publication WO97/34196, U.S. Pat. No. 5,686,228 or Japanese Patent Application Nos. 8-279962, 9-228881, 9-273935, 9-354107, 9-309813, 9-296174, 9-282564, 9-272002, 9-272003 and 9-332388 may also be used in combination.

In addition, the acrylonitrile compounds disclosed in U.S. Pat. No. 5,545,515, more specifically the compounds CN-1 to CN-13 disclosed therein and the like may also be used as the ultrahigh contrast agent.

In the present invention, a contrast accelerator may be used in combination with the above-described ultrahigh contrast agent for the formation of an ultrahigh contrast image. For example, amine compounds described in U.S.

Pat. No. 5,545,505, specifically, AM-1 to AM-5; hydroxamic acids described in U.S. Pat. No. 5,545,507, specifically, HA-1 to HA-11; hydrazine compounds described in U.S. Pat. No. 5,558,983, specifically, CA-1 to CA-6; and onium salts described in JP-A-9-297368, specifically, A-1 to A-42, B-1 to B-27 and C-1 to C-14 may be used.

Method for preparation and addition as well as amounts of the aforementioned ultrahigh contrast agents and the contrast accelerators may be applied as those described in the patent publications cited above.

The ultrahigh contrast agents preferably used in the present invention may be used after being dissolved in water or an appropriate organic solvent such as an alcohol (e.g., methanol, ethanol, propanol, fluorinated alcohol), a ketone (e.g., acetone, methyl ethyl ketone), dimethylformamide, dimethyl sulfoxide or methyl cellosolve. Alternatively, they may also be used as an emulsified dispersion mechanically prepared according to an already well known emulsification dispersion method by using an oil such as dibutyl phthalate, tricresyl phosphate, glyceryl triacetate or diethyl phthalate, ethyl acetate or cyclohexanone as an auxiliary solvent for dissolution. Alternatively, the ultrahigh contrast agents may be used after dispersion of them in powder form in water by using a ball mill, a colloid mill, or by means of ultrasonic wave according to a known method for solid dispersion.

The ultrahigh contrast agents used for the present invention may be added to any layers on the same side of a support as that provided with the aforementioned photosensitive silver halide and the reducible silver salt. However, the

compounds may preferably be added to a layer containing the silver halide or a layer adjacent thereto.

The heat-developable photosensitive material of the present invention preferably contains a reducing agent for organic silver salt. The reducing agent for organic silver salt may be any substance, preferably an organic substance, which reduces the silver ion to metal silver. Conventional photographic developers such as phenidone, hydroquinone and catechol are useful. The reducing agent is preferably contained in an amount of from 5 to 50% by mole, more preferably from 10 to 40% by mole based on per mole of silver on the surface having an image-forming layer. The layer to which the reducing agent is added may be any layer on the surface having an image-forming layer. Where the reducing agent is added to a layer other than the image-forming layer, the reducing agent is preferably used in a slightly large amount, i.e., from 10 to 50% by mole based on one mole of silver. The reducing agent may also be a so-called precursor that is modified so as to effectively exhibit the function only at the time of development.

For the heat-developable photosensitive material using an organic silver salt, variety of reducing agents can be used. For example, there can be used those reducing agents disclosed in JP-A-46-6074, JP-A-47-1238, JP-A-47-33621, JP-A-49-46427, JP-A-49-115540, JP-A-50-14334, JP-A-50-36110, JP-A-50-147711, JP-A-51-32632, JP-A-51-1023721, JP-A-51-32324, JP-A-51-51933, JP-A-52-84727, JP-A-55-108654, JP-A-56-146133, JP-A-57-82828, JP-A-57-82829, JP-A-6-3793, U.S. Pat. Nos. 3,667,9586, 3,679,426, 3,751,252, 3,751,255, 3,761,270, 3,782,949, 3,839,048, 3,928,686 and 5,464,738, German Patent No. 2,321,328, European Patent 692732 and the like. Examples include amidoximes such as phenylamidoxime, 2-thienylamidoxime and p-phenoxyphenylamidoxime; azines such as 4-hydroxy-3,5-dimethoxybenzaldehyde azine; combinations of an aliphatic carboxylic acid arylhydrazone with an ascorbic acid such as a combination of 2,2-bis(hydroxymethyl)propionyl- $\beta$ -phenylhydrazine with an ascorbic acid; combinations of polyhydroxybenzene with hydroxylamine, reductone and/or hydrazine such as a combination of hydroquinone with bis(ethoxyethyl)hydroxylamine, piperidinohexose reductone or formyl-4-methylphenylhydrazine; hydroxamic acids such as phenylhydroxamic acid, p-hydroxyphenylhydroxamic acid and  $\beta$ -anilinehydroxamic acid; combinations of an azine with a sulfonamidophenol such as a combination of phenothiazine with 2,6-dichloro-4-benzenesulfonamidophenol;  $\alpha$ -cyanophenylacetic acid derivatives such as ethyl- $\alpha$ -cyano-2-methylphenylacetate and ethyl- $\alpha$ -cyanophenylacetate; bis- $\beta$ -naphthols such as 2,2'-dihydroxy-1,1'-binaphthyl, 6,6'-dibromo-2,2'-dihydroxy-1,1'-binaphthyl and bis(2-hydroxy-1-naphthyl) methane; combinations of a bis- $\beta$ -naphthol with a 1,3-dihydroxybenzene derivative (e.g., 2,4-dihydroxybenzophenone, 2',4'-dihydroxyacetophenone); 5-pyrazolones such as 3-methyl-1-phenyl-5-pyrazolone; reductones such as dimethylaminohexose reductone, anhydriodihydroaminohexose reductone and anhydriodihydropiperidonehexose reductone; sulfonamidophenol reducing agents such as 2,6-dichloro-4-benzenesulfonamidophenol and p-benzenesulfonamidophenol; 2-phenylindane-1,3-diones; chromans such as 2,2-dimethyl-7-t-butyl-6-hydroxychroman; 1,4-dihydropyridines such as 2,6-dimethoxy-3,5-dicarboethoxy-1,4-dihydropyridine; ascorbic acid derivatives such as 1-ascorbyl palmitate and ascorbyl stearate; aldehydes and ketones such as benzyl and biacetyl; 3-pyrazolidone and a certain kind of indane-1,3-diones; and chromanols such as tocopherol.

Where the reducing agent is used in the present invention, the reducing agent may be added in any form, for example, as a solution, powder, solid fine grain dispersion and the like. The solid fine grain dispersion is performed using a known pulverizing means (e.g., a ball mill, a vibrating ball mill, a sand mill, a colloid mill, a jet mill, a roller mill). At the time of solid fine grain dispersion, a dispersion aid may also be used.

Furthermore, hydrazine derivatives may be preferably used as an ultrahigh contrast agent according to the present invention. For example, the hydrazine derivatives disclosed in Japanese Patent Application Nos. 9-166628, 8-279957 and 9-240511 may be used in combination with the anti-fogging of the present invention. In addition, the following 10 hydrazine derivatives may also be used in combination: the compounds represented by (Chem. 1) of JP-B-6-77138, specifically, compounds described at pages 3 and 4 of the publication; the compounds represented by the formula (I) of JP-B-6-93082, specifically, Compounds 1 to 38 described 15 at pages 8 to 18 of the publication; the compounds represented by the formulae (4), (5) and (6) of JP-A-6-230497, specifically, Compounds 4-1 to 4-10 described at pages 25 and 26, Compounds 5-1 to 5-42 described at pages 28 to 36 and Compounds 6-1 to 6-7 described at pages 39 and 40 of 20 the publication; the compounds represented by the formulae (1) and (17) of JP-A-6-289520, specifically, Compounds 1-1 to 1-17 and 2-1 described at pages 5 to 7 of the publication; the compounds represented by (Chem. 2) and (Chem. 3) of JP-A-6-313936, specifically, compounds described at pages 6 to 19 of the publication; the compound represented by (Chem. 1) of JP-A-6-313951, specifically, the compounds described at pages 3 to 5 of the publication; the compound represented by the formula (I) of JP-A-7-5610, specifically, Compounds I-1 to I-38 described at pages 25 25 to 10 of the publication; the compounds represented by the formula (II) of JP-A-7-77783, specifically, Compounds II-1 to II-102 described at pages 10 to 27 of the publication; the compounds represented by the formulae (H) and (Ha) of JP-A-7-104426, specifically, Compounds H-1 to H-44 described at pages 8 to 15 of the publication; the compounds characterized by having in the vicinity of the hydrazine group an anionic group or a nonionic group capable of forming an intramolecular hydrogen bond with a hydrogen atom of hydrazine, described in EP713131A, particularly, 30 the compounds represented by the formulae (A), (B), (C), (D), (E) and (F), specifically, Compounds N-1 to N-30 described in the publication; the compound represented by the formula (1) described in EP713131A, specifically, Compounds D-1 to D-55 described in the publication; various 35 hydrazine derivatives described at pages 25 to 34 of Kochi Gijutsu (Known Techniques), pages 1 to 207, Aztech (issued on Mar. 22, 1991); and Compounds D-2 and D-39 described in JP-A-62-86354 (pages 6 and 7).

The amount of the hydrazine derivatives is preferably 40 from  $1 \times 10^{-6}$  to 1 mol, more preferably from  $1 \times 10^{-5}$  to  $5 \times 10^{-1}$  mol, most preferably from  $2 \times 10^{-5}$  to  $2 \times 10^{-1}$  mol based on per mole of silver.

These hydrazine derivatives for use in the present invention may be used after being dissolved in an appropriate 45 organic solvent such as an alcohol (e.g., methanol, ethanol, propanol, fluorinated alcohol), a ketone (e.g., acetone, methyl ethyl ketone), dimethylformamide, dimethyl sulfoxide or methyl cellosolve. The compounds may also be used as an emulsified dispersion mechanically prepared according to an already well known emulsification dispersion method by using an oil such as dibutyl phthalate, tricresyl phosphate, glyceryl triacetate or diethyl phthalate, ethyl 50

acetate or cyclohexanone as an auxiliary solvent for dissolution. Alternatively, the compounds may be used after dispersion of a powder in water by using a ball mill, a colloid mill, or by means of ultrasonic wave according to a known method for solid dispersion.

The hydrazine derivatives may be added to any layers on a support provided that the layers are present on the same side as the surface provided with the aforementioned photosensitive silver halide and the reducible silver salt. However, they are preferably added to a layer containing the silver halide or a layer adjacent thereto.

In the heat-developable photosensitive material of the present invention, when an additive known as a "color-tone adjustor" capable of improving an image is added, an optical density may sometimes increase. The color-tone adjustor may also be sometimes advantageous in forming a black silver image. The color-tone adjustor may preferably be added in the surface having an image-forming layer in an amount of from 0.1 to 50% by mole, more preferably from 0.5 to 20% by mole based on one mole of silver. The color-tone adjustor may be a so-called precursor that is modified to effectively act only at the time of development.

For the heat-developable photosensitive material using an organic silver salt, a wide variety of color-tone adjustors can be used. For example, there can be used those color-tone adjustors disclosed in JP-A-46-6077, JP-A-47-10282, JP-A-49-5019, JP-A-49-5020, JP-A-49-91215, JP-A-49-91215, JP-A-50-2524, JP-A-50-32927, JP-A-50-67132, JP-A-50-67641, JP-A-50-114217, JP-A-51-3223, JP-A-51-27923, JP-A-52-14788, JP-A-52-99813, JP-A-53-1020, JP-A-53-76020, JP-A-54-156524, JP-A-54-156525, JP-A-61-183642, JP-A-4-56848, JP-B-49-10727, JP-B-54-20333, U.S. Pat. Nos. 3,080,254, 3,446,648, 3,782,941, 4,123,282 and 4,510,236, British Patent No. 1,380,795, Belgian Patent No. 841910 and the like. Examples of the color-tone adjustor include phthalimide and N-hydroxypythalimide; succinimide, pyrazolin-5-ones and cyclic imides such as quinazolinone, 3-phenyl-2-pyrazolin-5-one, 1-phenylurazole, quinazoline and 2,4-thiazolidinedione; naphthalimides such as N-hydroxy-1,8-naphthalimide; cobalt complexes such as cobalt hexaminetrifluoroacetate; mercaptanes such as 3-mercaptop-1,2,4-triazole, 2,4-dimercaptopyrimidine, 3-mercaptop-4,5-diphenyl-1,2,4-triazole and 2,5-dimercapto-1,3,4-thiadiazole; N-(aminomethyl)aryldicarboxyimides such as N,N-(dimethylamino-methyl)phthalimide and N,N-(dimethylaminomethyl)naphthalene-2,3-dicarboxyimide; blocked pyrazoles, isothiuronium derivatives and certain photobleaching agents, such as N,N'-hexamethylenebis(1-carbamoyl-3,5-dimethylpyrazole), 1,8-(3,6-diazaoctane)bis(iso-thiuronium trifluoroacetate) and 2-(tribromomethylsulfonyl)benzothiazole; 3-ethyl-5-[(3-ethyl-2-benzothiazolinylidene)-1-methylethylidene]-2-thio-2,4-oxazolidinedione; phthalazinone, phthalazinone derivatives and metal salts thereof, such as 4-(1-naphthyl)phthalazinone, 6-chlorophthalazinone, 5,7-dimethoxyphthalazinone or 2,3-dihydro-1,4-phthalazinedione; combinations of phthalazinone with a phthalic acid derivative such as phthalic acid, 4-methylphthalic acid, 4-nitrophthalic acid, and tetrachlorophthalic acid anhydride; phthalazine, phthalazine derivatives such as 4-(1-naphthyl)phthalazine, 6-chlorophthalazine, 5,7-dimethoxyphthalazine, 6-tert-butyl phthalazine, 5,7-dimethylphthalazine, and 2,3-dihydrophthalazine and metal salts thereof; combinations of a phthalazine and a phthalic acid derivative such as phthalic acid, 4-methylphthalic acid, 4-nitrophthalic acid, and tetra-

chlorophthalic acid anhydride; quinazolinedione, benzoxazine and naphthoxazine derivatives; rhodium complexes which function not only as a color-tone adjustor but as a halide ion source for the formation of silver halide at the site, such as ammonium hexachlororhodate(III), rhodium bromide, rhodium nitrate and potassium hexachlororhodate(III); inorganic peroxides and persulfates such as ammonium disulfide peroxide and hydrogen peroxide; benzoxazine-2,4-diones such as 1,3-benzoxazin-2,4-dione, 8-methyl-1,3-benzoxazin-2,4-dione, and 6-nitro-1,3-benzoxazin-2,4-dione; pyrimidines and asymmetric triazines such as 2,4-dihydroxypyrimidine and 2-hydroxy-4-aminopyrimidine; and azauracil and tetraazapentalene derivatives such as 3,6-dimercapto-1,4-diphenyl-1H,4H-2,3a,5,6-a-tetraazapentalene and 1,4-di(o-chlorophenyl)-3,6-dimercapto-1H,4H-2,3a,5,6a-tetraazapentalene and the like.

The color-tone adjustor may be added in any form, for example, as a solution, a powder, a solid fine grain dispersion and the like. The solid fine particle dispersion is performed using a known pulverization means (e.g., a ball mill, a vibrating ball mill, a sand mill, a colloid mill, a jet mill, a roller mill). At the time of solid fine grain dispersion, a dispersion aid may also be used.

As a sensitizing dye that can be used for the present invention, any sensitizing dyes may be used so long that they can spectrally sensitize the silver halide grains at a desired wavelength range when they adsorb on the silver halide particles. For example, there can be used cyanine dyes, merocyanine dyes, complex cyanine dyes, complex merocyanine dyes, holopolar cyanine dyes, styryl dyes, hemicyanine dyes, oxonole dyes, hemioxonole dyes and the like. Preferable sensitizing dyes which can be used in the present invention are described, for example, in Research Disclosure, Item 17643, IV-A (December, 1978, page 23), Item 1831X (August, 1978, page 437) and also in the references cited therein. In particular, sensitizing dyes having a spectral sensitivity suitable for spectral characteristics of light sources of various laser imagers, scanners, image setters, process cameras and the like can advantageously be chosen.

As examples of spectral sensitization to red light, for example, to so-called red light sources such as He-Ne laser, red semiconductor laser, LED and the like, Compounds I-1 to I-38 disclosed in JP-A-54-18726, Compounds I-1 to I-35 disclosed in JP-A-6-75322, Compounds I-1 to I-34 disclosed in JP-A-7-287338, Dyes 1 to 20 disclosed in JP-B-55-39818, Compounds I-1 to I-37 disclosed in JP-A-62-284343, Compounds I-1 to I-34 disclosed in JP-A-7-287338 and the like may be used.

To semiconductor laser light sources having a wavelength range of from 750 to 1,400 nm, spectral sensitization can be advantageously achieved by various known dyes including cyanine dyes, merocyanine dyes, styryl dyes, hemicyanine dyes, oxonol dyes, hemioxonol dyes and xanthene dyes. Useful cyanine dyes are cyanine dyes having a basic nucleus such as thiazoline nucleus, oxazoline nucleus, pyrroline nucleus, pyridine nucleus, oxazole nucleus, thiazole nucleus, selenazole nucleus or imidazole nucleus. Useful and preferred merocyanine dyes are merocyanine dyes having the above-described basic nucleus or an acidic nucleus such as thiohydantoin nucleus, rhodanine nucleus, oxazolidinedione nucleus, thiazolinedione nucleus, barbituric acid nucleus, thiazolinone nucleus, malononitrile nucleus or pyrazolone nucleus. The aforementioned cyanine and merocyanine dyes having an imino group or a carboxyl group are particularly effective. The dye may be appropriately chosen from known dyes described, for example, in U.S. Pat. Nos.

3,761,279, 3,719,495 and 3,877,943, British Patent Nos. 1,466,201, 1,469,117 and 1,422,057, JP-B-3-10391, JP-B-6-52387, JP-A-5-341432, JP-A-6-194781 and JP-A-6-301141.

The dyes that can most preferably be used for the present invention are cyanine dyes having one or more functional groups containing a thioether bond (e.g., cyanine dyes described in JP-A-62-58239, JP-A-3-138638, JP-A-3-138642, JP-A-4-255840, JP-A-5-72659, JP-A-5-72661, JP-A-6-222491, JP-A-2-230506, JP-A-6-258757, JP-A-6-317868, JP-A-6-324425, JP-W-A-7-500926 (the abbreviation "JP-W-A" as used herein means an "international application published in Japanese for Japanese national phase"), and U.S. Pat. No. 5,541,054), dyes having a carboxylic acid group (e.g., dyes disclosed in JP-A-3-163440, JP-A-6-301141, and U.S. Pat. No. 5,441,899), merocyanine dyes, polynuclear merocyanine dyes and polynuclear cyanine dyes (dyes disclosed in JP-A-47-6329, JP-A-49-105524, JP-A-51-127719, JP-A-52-80829, JP-A-54-61517, JP-A-59-214846, JP-A-60-6750, JP-A-63-159841, JP-A-6-35109, JP-A-6-59381, JP-A-7-146537, JP-A-7-146537, JP-A-W-55-50111, British Patent No. 1,467,638, and U.S. Pat. No. 5,281,515) and the like.

Dyes forming J-band are disclosed in U.S. Pat. Nos. 5,510,236, 3,871,887 (Example 5), JP-A-2-96131, JP-A-59-48753 and the like, and they can preferably be used for the present invention.

Each of these sensitizing dyes may be used alone or in any combination. A combination of sensitizing dyes is frequently used, especially for supersensitization. The emulsion may also contain, together with the sensitizing dye, a dye which itself does not have sensitizing effect or a substance which itself does not substantially absorb visible light, but shows supersensitization. Useful sensitizing dyes, combinations of dyes which exhibit supersensitization, and materials which show supersensitization are described in *Research Disclosure*, Vol. 176, 17643, page 23, Item IV-J (December, 1978), JP-B-49-25500, JP-B-43-4933, JP-A-59-19032, JP-A-59-192242 and the like.

The sensitizing dye may be added to the silver halide emulsion by dispersing the dye directly in the emulsion, or alternatively, the dye may be added to the emulsion after being dissolved in a single solvent or a mixed solvent chosen from water, methanol, ethanol, propanol, acetone, methyl cellosolve, 2,2,3,3-tetrafluoropropanol, 2,2,2-2-trifluoroethanol, 3-methoxy-1-propanol, 3-methoxy-1-butanol, 1-methoxy-2-propanol and N,N-dimethylformamide.

Furthermore, the sensitizing dye may be added according to the following methods: a method disclosed in U.S. Pat. No. 3,469,987 which comprises the step of dissolving a dye in a volatile organic solvent, dispersing the solution in water or hydrophilic colloid, and then adding the dispersion to an emulsion; a method disclosed in JP-B-44-23389, JP-B-44-27555 and JP-B-57-22091 which comprises the step of dissolving a dye in an acid, and adding the solution to an emulsion, or alternatively, preparing an aqueous solution in the presence of an acid or a base, and then adding the aqueous solution to an emulsion; a method disclosed in U.S. Pat. Nos. 3,822,135 and 4,006,025 which comprises the step of forming an aqueous solution or a colloid dispersion of a dye in the presence of a surface active agent, and then adding the solution or the dispersion to an emulsion; a method disclosed in JP-A-53-102733 and JP-A-58-105141 which comprises the step of dissolving a dye directly in hydrophilic colloid, and adding the dispersion to an emulsion; or a method disclosed in JP-A-51-74624 which comprises the

step of dissolving a dye using a compound capable of red shifting, and adding the solution to an emulsion. An ultrasonic wave may also be applied to dissolve the dye.

The sensitizing dye may be added to a silver halide emulsion in any steps heretofore known to be useful in the preparation of an emulsion. The sensitizing dye may be added at any time or in any step before the coating of the emulsion, for example, in the grain formation process of silver halide and/or before desalting or during the desalting process and/or the time period from desalting until initiation of chemical ripening, as disclosed in U.S. Pat. Nos. 2,735, 766, 3,628,960, 4,183,756 and 4,225,666, JP-A-58-184142 and JP-A-60-196749, or immediately before or during the chemical ripening process or in the time period after chemical ripening until coating, as disclosed in JP-A-58-113920. Furthermore, as disclosed in U.S. Pat. No. 4,225,666 and JP-A-58-7629, a single compound or a compound in combination with a structurally different compound may be added in divided portions, for example, one portion is added during grain formation and another is added during or after chemical ripening, or one portion is added before or during chemical ripening and another is added after completion of the chemical ripening. A type of a compound or a type of combination of compounds may be changed during the divided addition.

The amount of the sensitizing dye used may be appropriately chosen depending on the performance such as sensitivity or fog. The amount may preferably be from  $10^{-6}$  to 1 mol, more preferably from  $10^{-4}$  to  $10^{-1}$  mol based on one mole of silver halide in the photosensitive layer.

The heat-developable photosensitive material of the present invention may contain a mercapto compound, a disulfide compound or a thione compound, for example, to control the development by inhibition or acceleration, to improve spectral sensitization efficiency, and to improve storage stability before or after the development.

When a mercapto compound is used in the present invention, a mercapto compound having any chemical structure may be used, and those represented by Ar—SM or Ar—S—S—Ar are preferred, wherein M is a hydrogen atom or an alkali metal atom, and Ar is an aromatic ring or condensed aromatic ring containing one or more nitrogen, sulfur, oxygen, selenium or tellurium atoms. Preferably, the heteroaromatic ring may be benzimidazole, naphthimidazole, benzothiazole, naphthothiazole, benzoxazole, naphthoxazole, benzoselenazole, benzotellurazole, imidazole, oxazole, pyrazole, triazole, thiadiazole, tetrazole, triazine, pyrimidine, pyridazine, pyrazine, pyridine, purine, quinoline and quinazolinone. The heteroaromatic ring may have a functional group selected from, for example, the group consisting of halogen (e.g., Br, Cl), hydroxyl, amino, carboxyl, an alkyl group (e.g., alkyl having one or more carbon atoms, preferably from 1 to 4 carbon atoms), an alkoxy group (e.g., alkoxy having one or more carbon atoms, preferably from 1 to 4 carbon atoms), and an aryl group (which may have one or more functional groups). Examples of the mercapto substituted heteroaromatic compound include 2-mercaptopbenzimidazole, 2-mercaptopbenzoxazole, 2-mercaptopbenzothiazole, 2-mercaptop-5-methylbenzimidazole, 6-ethoxy-2-mercaptopbenzothiazole, 2,2-dithiobis(benzothiazole), 3-mercaptop-1,2,4-triazole, 4,5-diphenyl-2-imidazolethiol, 2-mercaptopimidazole, 1-ethyl-2-mercaptopbenzimidazole, 2-mercatoquinoline, 8-mercaptopurine, 2-mercato-4(3H)-quinazolinone, 7-trifluoromethyl-4-quinolinethiol, 2,3,5,6-tetrachloro-4-pyridinethiol, 4-amino-6-hydroxy-2-mercaptopurine monohydrate, 2-amino-5-mercaptop-1,

3,4-thiadiazole, 3-amino-5-mercaptop-1,2,4-triazole, 4-hydroxy-2-mercaptopurimidine, 2-mercaptopurimidine, 4,6-diamino-2-mercaptopurimidine, 2-mercaptop-4-methyl-purimidine hydrochloride, 3-mercaptop-5-phenyl-1,2,4-triazole, 1-phenyl-5-mercaptotetrazole, sodium 3-(5-mercaptopurimidine)benzenesulfonate, N-methyl-N'-{3-(5-mercaptopurimidyl)phenyl}urea, 2-mercaptop-4-phenyloxazole, N-[3-(mercaptopropanylamino)propyl]carbazole and the like. However, the present invention is not limited to these examples.

The amount of the mercapto compound may preferably be from 0.0001 to 1.0 mol, more preferably from 0.001 to 0.3 mol based on one mole of silver in the image-forming layer.

The image-forming layer (photosensitive layer) of the heat-developable photosensitive material of the present invention may contain, as a plasticizer or a lubricant, polyhydric alcohols (for example, glycerins and diols described in U.S. Pat. No. 2,960,404), fatty acids or esters described in U.S. Pat. Nos. 2,588,765 and 3,121,060, and silicone resins described in British Patent No. 955,061.

The image-forming layer of the heat-developable photosensitive material according to the present invention may contain a dye or a pigment of various types to improve color tone or prevent irradiation. Any dye or pigment may be used, and examples thereof include pigments and dyes described in the color index. Specific examples thereof include organic pigments and inorganic pigments such as pyrazoloazole dyes, anthraquinone dyes, azo dyes, azomethine dyes, oxonol dyes, carbocyanine dyes, styryl dyes, triphenylmethane dyes, indoaniline dyes, indophenol dyes and phthalocyanines. Preferred examples of the dye include anthraquinone dyes (e.g., Compounds 1 to 9 described in JP-A-5-341441, Compounds 3-6 to 3-18 and 3-23 to 3-38 described in JP-A-5-165147), azomethine dyes (e.g., Compounds 17 to 47 described in JP-A-5-341441), indoaniline dyes (e.g., Compounds 1 to 19 described in JP-A-5-289227, Compound 47 described in JP-A-5-341441, Compounds 2-10 and 2-11 described in JP-A-5-165147) and azo dyes (Compounds 10 to 16 described in JP-A-5-341441).

The amount of the dye or pigment may be determined depending on a desired amount of absorption. In general, the compound is preferably used in an amount of from 1  $\mu$ g to 1 g per square meter of the photosensitive material. These dye and pigment may be added in any form, for example, as a solution, emulsified product or solid fine grain dispersion, or as a dye mordanted with a polymer mordant.

The heat-developable photosensitive material of the present invention may have a surface protective layer, for example, to prevent adhesion of the image-forming layer.

The surface protective layer may contain any polymers as a binder. The surface protective layer may preferably contain a polymer having carboxyl residues in an amount of from 100 mg/m<sup>2</sup> to 5 g/m<sup>2</sup>. Examples of the polymer having carboxyl residues include, for example, natural polymers (e.g., gelatin, alginic acid), modified natural polymers (e.g., carboxymethyl cellulose, phthalized gelatin), synthetic polymers (e.g., polymethacrylate, polyacrylate, poly(alkyl methacrylate)/acrylate copolymer, polystyrene/polymethacrylate copolymer) and the like. The content of the carboxyl residue in the polymers is preferably from 10 mmol to 1.4 mol per 100 g of the polymer. The carboxylic acid residues may form salts with alkali metal ions, alkaline earth metal ions, organic cations and the like.

For the surface protective layer, any anti-adhesion material can be used. Examples of the anti-adhesion material include wax, silica particles, styrene-containing elastomeric block copolymer (e.g., styrene/butadiene/styrene, styrene/

isoprene/styrene), cellulose acetate, cellulose acetate butyrate, cellulose propionate and a mixture thereof. The surface protective layer may also contain a crosslinking agent for forming cross-linkage or a surface active agent for improving coating property.

In the heat-developable photosensitive material of the present invention, the image-forming layer or the protective layer for the image-forming layer may contain a light-absorbing material and a filter dye described in U.S. Pat. Nos. 3,253,921, 2,274,782, 2,527,583 and 2,956,879. The dyes can be mordanted as described, for example, U.S. Pat. No. 3,282,699. The filter dye is preferably used in such an amount that achieves absorbance at an exposure wavelength of from 0.1 to 3, most preferably from 0.2 to 1.5.

The heat-developable photosensitive material of the present invention is preferably a so-called single-sided photosensitive material comprising a support having on one side thereof at least one photosensitive layer containing a silver halide emulsion (preferably, an image-forming layer) and on the other side thereof a backing layer.

The backing layer preferably has a maximum absorption of from about 0.3 to 2.0 in a desired wavelength range. Where the desired range is from 750 to 1,400 nm, the backing layer may preferably have an optical density of from 0.005 to less than 0.5 at from 360 to 750 nm, and more preferably act as an antihalation layer having optical density of from 0.001 to less than 0.3. Where the desired range is less than 750 nm, the backing layer may preferably be an antihalation layer having a maximum absorption of from 0.3 to 2.0 in a desired range of wavelength before the formation of an image, and an optical density of from 0.005 to less than 0.3 at from 360 to 750 nm after the formation of an image. The method for decreasing the optical density after the formation of an image to the above-described range is not particularly limited. For example, a method for reducing the density through decoloration of a dye by heating as described in Belgian Patent No. 733,706, or a method for reducing the density using decoloration by light irradiation described in JP-A-54-17833 may be used.

When antihalation dyes are used, the dyes may be any compounds so far that they have an intended absorption in a desired wavelength region and sufficiently low absorption in a visible region, and also provide an absorption spectral property desired for the aforementioned backing layer. Examples of such dye include, as a single dye, the compounds described in JP-A-59-56458, JP-A-2-216140, JP-A-7-13295, JP-A-7-11432, U.S. Pat. No. 5,380,635, JP-A-2-68539 (from page 13, left lower column, line 1 to page 14, left lower column, line 9) and JP-A-3-24539 (from page 14, left lower column to page 16, right lower column); and as a dye which is decolored after the treatment, the compounds described in JP-A-52-139136, JP-A-53-132334, JP-A-56-501480, JP-A-57-16060, JP-A-57-68831, JP-A-57-101835, JP-A-59-182436, JP-A-7-36145, JP-A-7-199409, JP-B-48-33692, JP-A-B-50-16648, JP-B-2-41734 and U.S. Pat. Nos. 4,088,497, 4,283,487, 4,548,896 and 5,187,049. However, the scope of the present invention is not limited to these examples.

The binder suitable for the backing layer may be transparent or translucent, and generally colorless. Examples include natural polymers and synthetic resins including homopolymers and copolymers, and other film-forming media. Specific examples include, for example, gelatin, gum arabic, poly(vinyl alcohol), hydroxyethyl cellulose, cellulose acetate, cellulose acetate butyrate, poly(vinyl pyrrolidone), casein, starch, poly(methacrylic acid), poly(methyl methacrylate), poly(vinyl chloride), poly(methacrylic acid),

copoly(styrene-maleic anhydride), copoly(styrene-acrylonitrile), copoly(styrene-butadiene), poly(vinyl acetals) (e.g., poly(vinyl formal), poly(vinyl butyral)), poly(esters), poly(urethanes), phenoxy resin, poly(vinylidene chloride), poly(epoxides), poly(carbonates), poly(vinyl acetate), cellulose esters and poly(amides). The binder may be coated and formed after being dissolved in water or an organic solvent or in the form of an emulsion.

The heat-developable photosensitive material of the present invention may contain, in the surface protective layer for the photosensitive emulsion layer (preferably image-forming layer) and/or the backing layer or in the surface protective layer for the backing layer, a matting agent to improve transferability. The matting agent is, in general, a fine particle of a water-insoluble organic or inorganic compound. Any matting agent may be employed, and those well known in the art may be used, such as organic matting agents described in U.S. Pat. Nos. 1,939,213, 2,701, 245, 2,322,037, 3,262,782, 3,539,344 and 3,767,448, or inorganic matting agents described in U.S. Pat. Nos. 1,260, 772, 2,192,241, 3,257,206, 3,370,951, 3,523,022 and 3,769, 020. Specific examples of the organic compound which can be used as the matting agent include, for example, water-dispersible vinyl polymers such as polymethyl acrylate, polymethyl methacrylate (PMMA), polyacrylonitrile, acrylonitrile/α-methylstyrene copolymer, polystyrene, styrene/divinylbenzene copolymer, polyvinyl acetate, polyethylene carbonate and polytetrafluoroethylene; cellulose derivatives such as methyl cellulose, cellulose acetate and cellulose acetate propionate; starch derivatives such as carboxy starch, carboxynitrophenyl starch and urea/formaldehyde/starch reaction product; and gelatin hardened with a known hardening agent and hardened gelatin subjected to coacervation hardening so as to be a microcapsule hollow particle. Examples of the inorganic compound include, for example, silicon dioxide, titanium dioxide, magnesium dioxide, aluminum oxide, barium sulfate, calcium carbonate, silver chloride desensitized by a known method, silver bromide desensitized by a known method, glass, diatomaceous earth and the like. The matting agent may be used as a mixture of different substances as required. The size and shape of the matting agent are not particularly limited and the matting agent may have any particle size. A matting agent having a particle size of from 0.1 to 30  $\mu\text{m}$  may preferably used to carry out the present invention. The matting agent may have either a narrow or broad particle size distribution. However, the matting agent may greatly affect the haze of the photosensitive layer or surface gloss of a coated layer, and accordingly, the particle size, shape and particle size distribution may preferably be controlled to meet a desired purpose at the preparation of the matting agent or by mixing several matting agents.

The matting agent may preferably be incorporated in the outermost surface layer of the photosensitive material or a layer which functions as the outermost surface layer, or alternatively, in a layer close to the outer surface or a layer which acts as a so-called protective layer. The matting degree on the surface protective layer for the emulsion layer can be freely chosen so far that the star dust trouble does not occur. The degree may preferably be within a range of from 500 to 10,000 seconds, most preferably from 500 to 2,000 seconds as indicated by the Beck's smoothness.

According to the present invention, the heat-developable photosensitive material that is a single-sided photosensitive material and has a backing layer containing a matting agent constitutes a preferred embodiment. The matting degree of the backing layer is from 10 to 1,200 seconds, more preferably from 50 to 700 seconds as indicated by the Beck's smoothness.

The heat-developable photographic emulsion for use in the present invention is coated on a support to form one or more layers. In the case of a single layer, the layer must contain an organic silver salt, a silver halide, a developer, a binder, and optionally added materials such as a color-tone adjustor, a coating aid and other auxiliary agents. In the case of a double-layer structure, the first emulsion layer (usually a layer adjacent to the substrate) must contain an organic silver salt and a silver halide, and the second layer or both layers must contain some other components. A double-layer structure comprising a single emulsion layer containing all of the components and a protective topcoat may also be contemplated. A multi-color photosensitive heat-developable photosensitive material may have the combination of the above-described two layers for each of the colors, or as described in U.S. Pat. No. 4,708,928, a structure comprising a single layer containing all components. In the case of a multi-dye multi-color photosensitive heat-developable material, a functional or non-functional barrier layer is generally provided between respective emulsion layers (photosensitive layers) to keep the emulsion layer away from each other as described in U.S. Pat. No. 4,460,681.

A backside resistive heating layer described in U.S. Pat. Nos. 4,460,681 and 4,374,921 may also be used in the photosensitive heat-developable photographic image system.

In the heat-developable photosensitive material of the present invention, a hardening agent may be used in layers such as the image-forming layer (photosensitive layer), the protective layer, and the backing layer. Examples of the hardening agent include polyisocyanates described in U.S. Pat. No. 4,281,060 and JP-A-6-208193, epoxy compounds described in U.S. Pat. No. 4,791,042, and vinyl sulfone-based compounds described in JP-A-62-89048.

In the heat-developable photosensitive material of the present invention, a surface active agent may also be used to improve the coating property and or electrostatic charge property. Examples of the surface active agent include nonionic, anionic, cationic and fluorocarbon surface active agents, which may be appropriately chosen and used. Specific examples include fluorocarbon polymer surface active agents described in JP-A-62-170950 and U.S. Pat. No. 5,380,644, fluorocarbon surface active agents described in JP-A-60-244945 and JP-A-63-188135, polysiloxane-based surface active agents described in U.S. Pat. No. 3,885,965, and polyalkylene oxides and anionic surface active agents described in JP-A-6-301140.

A support of various types can be used for the heat-developable photosensitive material of the present invention. Typical examples of the support include polyester film, undercoated polyester film, poly(ethylene terephthalate) film, polyethylene naphthalate film, nitrocellulose film, cellulose ester film, poly(vinyl acetal) film, polycarbonate film, related or resinous material, glass, paper and metal. A flexible substrate, particularly, a paper support coated with baryta and/or partially acetylated  $\alpha$ -olefin polymer, preferably, an  $\alpha$ -olefin polymer having 2 to 10 carbon atoms, such as polyethylene, polypropylene or ethylene/butene copolymer may typically be used. The support may be either transparent or opaque, and preferably be transparent. Among them, a biaxially stretched polyethylene terephthalate having a thickness of approximately from 75 to 200  $\mu\text{m}$  is particularly preferred.

When a plastic film is passed through a heat-developing apparatus and processed at 80° C. or higher, the film is generally stretched in the dimension. If the processed mate-

rials are used as printing photographic materials, the stretch causes a serious problem at the time of precision multi-color printing. Accordingly, in the present invention, it is preferred to use a film designed to cause little change in the dimension by relaxing the internal strain remaining in the film at the biaxial stretching and thereby eliminating the heat shrinkage distortion generated during the heat development. For example, polyethylene terephthalate heat-treated at 100 to 210° C. before a heat-developable photographic emulsion is coated thereon is preferably used. A film having a high glass transition point is also preferred, for example, a film of polyether ethyl ketone, polystyrene, polysulfone, polyether sulfone, polyarylate or polycarbonate may be used.

For the purpose of preventing the electrostatic charge, the heat-developable photosensitive material of the present invention may comprise a metallized layer or a layer containing a soluble salt (e.g., chloride, nitrate), an ionic polymer described in U.S. Pat. Nos. 2,861,056 and 3,206,313, an insoluble inorganic salt described in U.S. Pat. No. 3,428,451, or tin oxide fine particles described in JP-A-60-252349 and JP-A-57-104931.

To obtain a color image by using the heat-developable photosensitive material of the present invention, the method described in JP-A-7-13295, from page 10, left column, line 43 to page 11, left column, line 40 may be applied. Examples of a stabilizer for a color dye image include those described in British Patent 1,326,889, U.S. Pat. Nos. 3,432,300, 3,698,909, 3,574,627, 3,573,050, 3,764,337 and 4,042,394.

The heat-developable photographic emulsion for use in the present invention may be coating by various coating operations such as dip coating, air knife coating, flow coating or extrusion coating using a hopper such as described in U.S. Pat. No. 2,681,294. If desired, two or more layers may be simultaneously coated by a method described in U.S. Pat. No. 2,761,791 and British Patent No. 837,095.

The heat-developable photosensitive material of the present invention may comprise additional layers such as a dye-accepting layer for accepting a moving dye image, an opaque layer for the case of reflective printing, a protective topcoat layer or a primer layer known in the field of photothermic photographic technology. The photosensitive material of the present invention is preferably designed so that an image can be formed by the photosensitive material alone, although a functional layer necessary to form an image, such as an image-receiving layer, may be prepared as a separate photographic material.

The heat-developable photosensitive material of the present invention may be developed by any method. The development is usually performed by elevating the temperature of the photographic material after imagewise exposure. Preferred embodiments of the heat-developing apparatus include, as a type of contacting a heat-developable photosensitive material with a heat source such as heat roller or heat drum, the heat-developing apparatuses described in JP-B-5-56499, Japanese Patent No. 684453, JP-A-9-292695, JP-A-9-297385 and International Patent Publication WO95/30934, and as a non-contacting type, the heat-developing apparatuses described in JP-A-7-13294, International Patent publications WO97/28489, WO97/28488 and WO97/28287. A non-contacting type heat-developing apparatus is particularly preferred. The development temperature may preferably be from 80 to 250° C., more preferably from 100 to 140° C. The development time may preferably be from 1 to 180 seconds, more preferably from 10 to 90 seconds.

For preventing uneven processing of the heat-developable photosensitive material due to the change in the dimension

at the time of heat development, a method comprising the steps of heating the photographic material at a temperature of from 80° C. to less than 115° C. (preferably 113° C. or lower) for 5 seconds or more so that an image is not formed, and then heat-developing the material at 110° C. or higher (preferably 130° C. or lower) to form an image (the so-called multi-stage heating method) is effective.

The heat-developable photosensitive material of the present invention may be light-exposed by any method. A preferable light source for the exposure is a laser ray. The laser ray for use in the present invention is preferably a gas laser, YAG laser, dye laser, semiconductor laser or the like. The semiconductor laser and a second harmonic generation device may be used in combination.

The heat-developable photosensitive material of the present invention has a low haze at the exposure and may sometimes generate interference fringes. For preventing the generation of interference fringes, a technique disclosed in JP-A-5-113548 which comprises the step of entering a laser ray obliquely in the photographic material, and a method of using a multimode laser disclosed in International Patent Publication WO95/31754 are known, and these techniques are preferably used.

The heat-developable photosensitive material of the present invention is preferably exposed in such a manner that laser rays overlap and the scanning lines are not observed as described in SPIE, Vol. 169, "Laser Printing", pages 116 to 128 (1979), JP-A-4-51043 and International Patent Publication WO95/31754.

An example of the structure of a heat-developing apparatus used for the heat development of the heat-developable photosensitive material of the present invention is shown in FIG. 1. FIG. 1 depicts a side view of a heat-developing apparatus. The apparatus shown in FIG. 1 comprises carrying-in roller pairs 11 (lower rollers are heating rollers), which carry a heat-developable photosensitive material 10 into the heating section while making the material in a flat shape and preheating it, and carrying-out roller pairs 12, which carry out the heat-developable photosensitive material 10 after heat development from the heating section while maintaining the material to be in a flat shape. The heat-developable photosensitive material 10 is heat-developed while it is conveyed by the carrying-in roller pairs 11 and then by the carrying-out roller pairs 12. A conveying means for carrying the heat-developable photosensitive material 10 under the heat development is provided with multiple rollers 13 so that they should be contacted with the side of the image-forming layer, and a flat surface 14 consisting of non-woven fabric (composed of aromatic polyamide, Teflon etc.) or the like is provided on the opposite side so that it should be contacted with the back surface. The heat-developable photosensitive material 10 is conveyed by driving of the multiple rollers 13 contacted with the image-forming layer side, while the back surface slides on the flat surface 14. As a heating means, heaters 15 are provided over the rollers 13 and under the flat surface 14 so that the heat-developable photosensitive material 10 should be heated from the both sides. Examples of the heating means include panel heaters and so forth. While clearance between the rollers 13 and the flat surface 14 may vary depending on the member of the flat surface, it is suitably adjusted to a clearance that allows the conveyance of the heat-developable photosensitive material 10. The clearance is preferably 0-1 mm.

The material of the surface of the rollers 13 and the member of the flat surface 14 may be composed of any materials so long as they have heat resistance and they

should not cause any troubles in the conveyance of the heat-developable photosensitive material 10. However, the material of the roller surface is preferably composed of silicone rubber, and the member of the flat surface is preferably composed of non-woven fabric made of aromatic polyamide or Teflon (polytetrafluoroethylene). The heating means preferably comprises multiple heaters so that temperature of each heater can be adjusted freely.

The heating section is constituted by a preheating section A comprising the carrying-in roller pairs 11 and a heat developing section B comprising the heaters 15. The temperature of the preheating section A located upstream of the heat developing section B is preferably selected to be lower than the heat development temperature (for example, by about 10–30°C.), and the temperature and heat development time are desirably adjusted so that they are sufficient for evaporating moisture contained in the heat-developable photosensitive material 10. The temperature of the heat developing section B is also preferably selected to be higher than the glass transition temperature (Tg) of the support of the heat-developable photosensitive material 10 so that uneven development should be prevented.

Moreover, guide panels 16 are provided downstream from the heat developing section B, and they constitute a slow cooling section C together with the carrying-out roller pairs 12.

The guide panels 16 are preferably composed of a material of low heat conductivity, and it is preferred that the cooling is performed slowly.

The heat-development apparatus is explained with reference to an example shown in the drawing. However, the apparatus is not limited to the example. For example, the heat-development apparatus used for the present invention may have a variety of structures such as disclosed in JP-A-7-13294. For the multi-stage heating method, which is preferably used in the present invention, the heat-developable photosensitive material may be successively heated at different temperatures in such an apparatus as mentioned above, which is provided with two or more heat sources at different temperatures.

#### EXAMPLES

The present invention will be specifically explained with reference to the following examples. Materials, reagents, ratios, operations and so forth can be suitably modified without deviating from the spirit of the present invention. Therefore, the scope of the present invention is not limited to the following examples.

##### Example 1

###### <<Preparation of PET Support>>

PET having IV (intrinsic viscosity) of 0.66 (measured in phenol/tetrachloroethane=6/4 (weight ratio) at 25°C.) was obtained by using terephthalic acid and ethylene glycol in a conventional manner. The product was pelletized, dried at 130°C. for 4 hours, then melted at 300°C., and extruded from a T-die and rapidly cooled to form an unstretched film having a thickness of 175 µm after thermal fixation.

The film was stretched along the longitudinal direction by 3.3 times at 110°C. using rollers of different peripheral speeds, and then stretched along the transverse direction by 4.5 times at 130°C. using a tenter. Then, the film was subjected to thermal fixation at 240°C. for 20 seconds, and relaxed by 4% along the transverse direction at the same temperature. Then, the chuck of the tenter was released, the both edges of the film were knurled, and the film was rolled up at 4.8 kg/cm<sup>2</sup>. Thus, a roll of a film having a thickness of 175 µm was obtained.

###### <<Surface Corona Discharge Treatment>>

The both surfaces of the support were subjected to corona discharge treatment at room temperature at a speed of 20 m/minute by using a solid state corona processor Model 6 5 KVA (manufactured by Piller Co., Ltd.). The readings of electric current and voltage during the treatment indicated that the support underwent the treatment of 0.375 kV·A-minute/m<sup>2</sup>. The discharging frequency of the treatment was 9.6 kHz, and the gap clearance between the 10 electrode and the dielectric roll was 1.6 mm.

###### <<Preparation of Support with Undercoat Layer>>

###### (Preparation of Coating Solution for Undercoat Layer A)

A polyester copolymer aqueous dispersion, Pesresin A-515GB (30%, 200 ml, Takamatsu Yushi KK) was added 15 with polystyrene microparticles (1 g, average particle diameter of 0.2 µm) and Surface active agent 1 (1 wt %, 20 ml), and added with distilled water to a volume of 1000 ml to form Coating solution for undercoat layer A.

###### (Preparation of Coating Solution for Undercoat Layer B)

Distilled water (680 ml) was added with a styrene/butadiene copolymer aqueous dispersion (styrene/butadiene/itaconic acid=47/50/3 [weight ratio], 200 ml, concentration: 30 wt %) and polystyrene microparticles (0.1 g, average particle diameter of 2.5 µm), and further added with 25 distilled water to a volume of 1000 ml to form Coating solution for undercoat layer B.

###### (Preparation of Coating Solution for Undercoat Layer C)

Inert gelatin (10 g) was dissolved in distilled water (500 ml), added with an aqueous dispersion (40 wt %, 40 g) of tin 30 oxide antimony oxide complex fine grains disclosed in JP-A-61-20033, and further added with distilled water to a volume of 1000 ml to form Coating solution for undercoat layer C.

###### (Preparation of Support with Undercoat Layer)

After the aforementioned corona discharge treatment, Coating solution for undercoat layer A was applied on the support by a bar coater in a wet amount of 5 ml/m<sup>2</sup>, and dried for 5 minutes at 180°C. The dry thickness was about 0.3 µm. Then, the opposite surface (back surface) was 35 subjected to the corona discharge treatment, applied with Coating solution for undercoat layer B by a bar coater in a wet coating amount of 5 ml/m<sup>2</sup> so as to obtain a dry thickness of about 0.3 µm, and dried for 5 minutes at 180°C. The coated layer was further applied with Coating 40 solution for undercoat layer C by a bar coater in a wet coating amount of 3 ml/m<sup>2</sup> so as to obtain a dry thickness of about 0.03 µm, and dried for 5 minutes at 180°C. to obtain a support with undercoat layers.

###### <<Preparation of Organic acid Silver Salt Dispersion>>

To a stirred mixture of behenic acid (43.8 g, product name: Edenor C22 85R, Henkel Corp.), distilled water (730 ml) and tert-butanol (60 ml) at 79°C., an aqueous 1N NaOH solution (117 ml) was added over 55 minutes, and allowed to react for 240 minutes. Then, the mixture was added with 55 an aqueous solution (112.5 ml) of silver nitrate (19.2 g) over 45 seconds, and left as it was for 20 minutes so that the temperature of the mixture was lowered to 30°C. Thereafter, the solid content was separated by suction filtration, and washed with water until the conductivity of the filtrate became 30 µS/cm. The solid content obtained as described above was not dried but handled as a wet cake. To this wet cake corresponding to 100 g of dry solid content, 7.4 g of polyvinyl alcohol (trade name: PVA205) and water were added to make the total amount of 385 g, and the resulting mixture was preliminarily dispersed in a homomixer.

Then, the preliminarily dispersed stock solution was treated three times in a dispersing machine (trade name:

Microfluidizer M-110S-EH, manufactured by Microfluidex International Corporation, using G10Z interaction chamber) under a pressure controlled to be 1,750 kg/cm<sup>2</sup> to obtain Silver behenate dispersion B. The silver behenate particles contained in the silver behenate dispersion obtained as described above were acicular grains having an average short axis length of 0.04  $\mu\text{m}$ , average long axis length of 0.8  $\mu\text{m}$  and variation coefficient of 30%. The grain size was measured by Master Sizer X manufactured by Malvern Instruments Ltd. During the cooling operation, a desired dispersion temperature was established by providing coiled heat exchangers fixed before and after the interaction chamber and controlling the temperature of the refrigerant.

## &lt;&lt;Preparation of 25 wt % Dispersion of Reducing Agent&gt;&gt;

To a phenol compound of the present invention (each compound shown in Table 1, 80 g) and a 20 wt % aqueous solution of denatured polyvinyl alcohol MP-203 produced by Kuraray Co., Ltd. (64 g), water (176 g) was added, and thoroughly stirred to obtain a slurry. The slurry was introduced into a vessel together with zirconia beads having an average diameter of 0.5 mm (800 g), and dispersed in a dispersing machine (1/4G Sand Grinder Mill, manufactured by Imex) for 5 hours to prepare a reducing agent dispersion. The reducing agent particles contained in the reducing agent dispersion had an average particle size of 0.72  $\mu\text{m}$ .

## &lt;&lt;Preparation of 20 wt % Dispersion of Mercapto Compound&gt;&gt;

To 3-mercaptopro-4-phenyl-5-heptyl-1,2,4-triazole (64 g) and a 20 wt % aqueous solution of denatured polyvinyl alcohol MP-203 produced by Kuraray Co., Ltd. (32 g), water (224 g) was added, and thoroughly stirred to obtain a slurry. The slurry was introduced into a vessel together with zirconia beads having an average diameter of 0.5 mm (800 g), and dispersed in a dispersing machine (1/4G Sand Grinder Mill, manufactured by Imex) for 10 hours to obtain a mercapto compound dispersion. The mercapto compound particles contained in the mercapto compound dispersion obtained as described above had an average particle size of 0.67  $\mu\text{m}$ .

## &lt;&lt;Preparation of 30 wt % Dispersion of Organic Polyhalogenated Compound&gt;&gt;

2-Tribromomethylsulfonylnaphthalene (116 g), a 20 wt % aqueous solution of denatured polyvinyl alcohol MP203 produced by Kuraray Co., Ltd. (48 g) and water (224 g) were thoroughly stirred to obtain a slurry. The slurry was introduced into a vessel together with zirconia beads having an average diameter of 0.5 mm (800 g), and dispersed in a dispersing machine (1/4G Sand Grinder Mill, manufactured by Imex) for 5 hours to obtain a dispersion of organic polyhalogenated compound. The organic polyhalogenated compound particles contained in the dispersion of organic polyhalogenated compound dispersion obtained as described above had an average particle size of 0.74  $\mu\text{m}$ .

## &lt;&lt;Preparation of Methanol Solution of Phthalazine Compound&gt;&gt;

6-Isopropylphthalazine (26 g) was dissolved in methanol (100 ml) and used.

## &lt;&lt;Preparation of 20 wt % Dispersion of Pigment&gt;&gt;

To C.I. Pigment Blue 60 (64 g) and Demor N produced by Kao Corporation (6.4 g), water (250 g) was added, and thoroughly stirred to obtain a slurry. The slurry was introduced into a vessel together with zirconia beads having an average diameter of 0.5 mm (800 g), and dispersed in a dispersing machine (1/4G Sand Grinder Mill, manufactured by Imex) for 25 hours to obtain a pigment dispersion. The pigment particles contained in the pigment dispersion obtained as described above had an average particle size of 0.21  $\mu\text{m}$ .

## &lt;&lt;Preparation of Silver Halide Grain 1&gt;&gt;

Distilled water (1421 ml) was added with a 1 wt % potassium bromide solution (6.7 ml), and further added with 1 N nitric acid (8.2 ml) and phthalized gelatin (21.8 g). Separately, Solution a1 was prepared by adding distilled water to silver nitrate (37.04 g) to dilute it to 159 ml, and Solution b1 was prepared by diluting potassium bromide (32.6 g) with distilled water to a volume of 200 ml. To the aforementioned mixture maintained at 35° C. and stirred in a titanium-coated stainless steel reaction vessel, the whole volume of Solution a1 was added by the controlled double jet method over minute at a constant flow rate while pAg was maintained at 8.1 (Solution b1 was also added by the controlled double jet method). Then, the mixture was added with 3.5 wt % aqueous hydrogen peroxide solution (30 ml), and further added with a 3wt % aqueous solution of benzimidazole (336 ml). Separately, Solution a2 was prepared by diluting Solution a1 with distilled water to a volume of 317.5 ml, and Solution b2 was prepared by dissolving dipotassium hexachloroiodate in Solution b1 in such an amount that its final concentration should be  $1\times 10^{-4}$  mol per mole of silver, and diluting the obtained solution with distilled water to a volume twice as much as the volume of Solution b1, 400 ml. The whole volume of Solution a2 was added to the mixture again by the controlled double jet method over 10 minutes at a constant flow rate while pAg was maintained at 8.1 (Solution b2 was also added by the controlled double jet method). Then, the mixture was added with a 0.5 wt % solution of 2-mercaptopro-5-methylbenzimidazole in methanol (50 ml). After pAg was raised to 7.5 with silver nitrate, the mixture was adjusted to pH 3.8 using 1 N sulfuric acid, and the stirring was stopped. Then, the mixture was subjected to precipitation, desalting and washing with water, added with deionized gelatin (3.5 g) and 1 N sodium hydroxide to be adjusted to pH 6.0 and pAg of 8.2 to form a silver halide dispersion.

The grains in the completed silver halide emulsion were pure silver bromide grains having an average spherical diameter of 0.031  $\mu\text{m}$  and a variation coefficient of 11% in terms of spherical diameter. The grain size and the like were obtained from averages for 1000 grains by using an electron microscope. The [100] face ratio of these grains were determined to be 85% by the Kubelka-Munk method.

The aforementioned emulsion was warmed to 50° C. with stirring, added with a 0.5 wt % solution of N,N-dihydroxy-N,N-diethylmelamine in methanol (5 ml) and a 3.5 wt % solution of phenoxyethanol in methanol (5 ml), and further added 1 minute later with sodium benzenethiosulfonate in an amount of  $3\times 10^{-5}$  mol per mole of silver. Further 2 minutes later, the emulsion was added with a solid dispersion of Spectral sensitization dye 1 (aqueous gelatin solution) in an amount of  $5\times 10^{-3}$  mol per mole of silver, added further 2 minutes later with a tellurium compound in an amount of  $5\times 10^{-5}$  mol per mole of silver, and ripened for 50 minutes. Immediately before the completion of the ripening, the emulsion was added with 2-mercaptopro-5-methylbenzimidazole in an amount of  $1\times 10^{-3}$  mol per mole of silver, and its temperature was lowered. Thus, chemical sensitization was finished to form Silver halide grain 1.

## &lt;&lt;Preparation of Silver Halide Grain 2&gt;&gt;

In 700 ml of water, phthalized gelatin (22 g) and potassium bromide (30 mg) were dissolved, and after adjusting the pH to 5.0 at a temperature of 35° C., an aqueous solution (159 ml) containing silver nitrate (18.6 g) and ammonium nitrate (0.9 g) and an aqueous solution containing potassium bromide and potassium iodide at a molar ratio of 92:8 were added by the control double jet method over 10 minutes

while pAg was maintained at 7.7. Subsequently, 476 ml of an aqueous solution containing silver nitrate (55.4 g) and ammonium nitrate (2 g) and an aqueous solution containing  $1 \times 10^{-5}$  mol of dipotassium hexachloroiridate and 1 mol of potassium bromide were added by the control double jet method over 30 minutes while pAg was maintained at 7.7, and then 4-hydroxy-6-methyl-1,3,3a,7-tetrazaaindene (1 g) was added. Then, pH of the mixture was lowered to cause coagulation precipitation to effect desalting, and the mixture was added with phenoxyethanol (0.1 g) and adjusted to pH 5.9 and pAg of 8.2 to complete the preparation of silver iodobromide grains (cubic grains having a core iodine content of 8 mol %, an average iodine content of 2 mol %, an average grain size of  $0.05 \mu\text{m}$ , a variation coefficient of the projected area of 8%, and a [100] face ratio of 88%).

The silver halide grains obtained above was warmed to  $60^\circ\text{C}$ ., added with sodium thiosulfonate in an amount of  $85 \mu\text{M}$  per mole of silver and 2,3,4,5,6-pentafluorophenylidiphenylphosphine selenide in an amount of  $1.1 \times 10^{-5}$  mol, a tellurium compound in an amount of  $1.5 \times 10^{-5}$  mol, chloroauric acid in an amount of  $3.5 \times 10^{-8}$  mol and thiocyanic acid in an amount of  $2.7 \times 10^{-4}$  mol, ripened for 120 minutes, then quenched to  $40^\circ\text{C}$ ., added with  $1 \times 10^{-4}$  mol of Spectral sensitization dye 1 and  $5 \times 10^{-4}$  mol of 2-mercapto-5-methylbenzimidazole, and quenched to  $30^\circ\text{C}$ . to obtain Silver halide emulsion 2.

**<<Preparation of Coating Solution for Emulsion Layer>>**  
**(Coating Solution for Emulsion Layer)**

The organic acid silver salt dispersion obtained above (103 g) and a 20 wt % aqueous solution of polyvinyl alcohol (5 g, PVA205, Kraray Co., Ltd.) were mixed and maintained at  $40^\circ\text{C}$ . To this mixture, a 10 wt % solution of a coupler compound (each compound shown in Table 1,  $1.0 \times 10^{-2}$  Mol per mole of silver) in DMF, the aforementioned 25 wt % reducing agent dispersion (23.2 g), the 5 wt % aqueous dispersion of the pigment, C.I. Pigment Blue 60 (4.8 g), the 30 wt % dispersion of organic polyhalogenated compound (10.7 g) and the 20 wt % mercapto compound dispersion (3.1 g) were added. Then, the mixture was added with a 40 wt % SBR latex (106 g) subjected to UF purification and maintained at  $40^\circ\text{C}$ ., and stirred sufficiently. The mixture was further added with the solution of phthalazine compound in methanol (6 ml) to obtain an organic acid silver salt solution. Moreover, Silver halide grain 1 (5 g) and Silver halide grain 2 (5 g) were sufficiently mixed beforehand, mixed with the organic acid silver salt dispersion by a static mixer immediately before application and used as a coating solution for emulsion layer. This coating solution was fed as it was to a coating die in such a feeding amount that a coated silver amount of  $1.4 \text{ g/m}^2$  should be obtained.

The viscosity of the aforementioned coating solution for emulsion layer was measured by a Brookfield viscometer of Tokyo Keiki, and found to be 85 [mPa·s] at  $40^\circ\text{C}$ . (No. 1 rotor).

The viscosity of the coating solution was measured at  $25^\circ\text{C}$ . by an RFS fluid spectrometer produced by Rheometric Far East Co., Ltd., and found to be 1500, 220, 70, 40 and 20 [mPa·s] at shear rates of 0.1, 1, 10, 100 and 1000 [1/second], respectively.

The SBR latex purified by UF (ultrafiltration) was obtained as follows. The following SBR latex diluted 10 times with distilled water was diluted and purified by using an UF purification module FS03 FC FUY03A1 (Daisen Membrane System Ltd.) until its ionic conductivity became 1.5 mS/cm and used. The latex concentration at that ionic conductivity was 40 wt %.

(SBR latex: latex of St(68) Bu(29) AA(3))

Average diameter of  $0.1 \mu\text{m}$ , concentration of 45 wt %, equilibrated moisture content ( $25^\circ\text{C}$ , 60% RH) of 0.6 wt %, ionic conductivity of 4.2 mS/cm (ionic conductivity was measured by using a conductometer CM-30S manufactured by Toa Electronics, Ltd. for a latex stock solution (40 wt %) at  $25^\circ\text{C}$ .), pH 8.2.

**<<Preparation of Coating Solution for Intermediate Layer on Emulsion Layer Side>>**

**10 (Coating Solution for Intermediate Layer)**

To 772 g of a 10 wt % aqueous solution of polyvinyl alcohol PVA205 (Kuraray Co., Ltd.), and 226 g of a 27.5 wt % latex of methyl methacrylate/styrene/2-ethylhexyl acrylate/hydroxyethyl methacrylate/acrylic acid copolymer (copolymerization weight ratio=59/9/26/5/1), a 5 wt % aqueous solution of Aerosol OT (American Cyanamid Co., 2 ml), benzyl alcohol (4 g), 2,2,4-trimethyl-1,3-pentanediol monoisobutyrate (1 g) and benzisothiazolinone (10 mg) were added to form a coating solution for intermediate layer, and fed to a coating die at such a feeding rate that its coating amount should be  $5 \text{ ml/m}^2$ .

The viscosity of the coating solution was measured by a Brookfield viscometer, and found to be 21 [mPa·s] at  $40^\circ\text{C}$ . (No. 1 rotor).

**25 <<Preparation of Coating Solution for First Protective Layer for Emulsion Layer>>**

**(Coating Solution for First Protective Layer)**

Inert gelatin (80 g) was dissolved in water, added with a 10 wt % solution of phthalic acid in methanol (138 ml), 1 N 30 sulfuric acid (28 ml), a 5 wt % aqueous solution (5 ml) of Aerosol OT (American Cyanamid Co.) and phenoxyethanol (1 g), and further added with water so that the total amount should be 1000 g to form a coating solution, which was fed to a coating die at such a feeding amount that its coating 35 amount should be  $10 \text{ ml/m}^2$ .

The viscosity of the coating solution was measured by a Brookfield viscometer, and found to be 17 [mPa·s] at  $40^\circ\text{C}$ . (No. 1 rotor).

**40 <<Preparation of Coating Solution for Second Protective Layer for Emulsion Layer>>**

**(Coating Solution for Second Protective Layer)**

Inert gelatin (100 g) was dissolved in water, added with a 5 wt % solution of N-perfluoroctylsulfonyl-N-propylalanine potassium salt (20 ml), a 5 wt % solution (16 ml) of Aerosol OT (American Cyanamid Co.), polymethyl 45 methacrylate microparticles (average diameter:  $4.0 \mu\text{m}$ , 25 g), 1 N sulfuric acid (44 ml) and benzisothiazolinone (10 mg), and further added with water to a total amount of 1555 g. The mixture was mixed with 445 ml of an aqueous 50 solution containing 4 wt % of chromium alum and 0.67 wt % of phthalic acid by a static mixer immediately before application and used as a coating solution for surface 55 protective layer. The coating solution was fed to a coating die in such an amount that the coating amount should be  $10 \text{ ml/m}^2$ .

The viscosity of the coating solution was measured by a Brookfield viscometer, and found to be 9 [mPa·s] at  $40^\circ\text{C}$ . (No. 1 rotor).

**<<Preparation of Coating Solutions for Back Surface>>**

**60 (Preparation of base Precursor Solid Fine Grain Dispersion)**

A base precursor compound (64 g) and a surface active agent (Demor N, Kao Corp., 10 g) were mixed with distilled water (246 ml), and the mixture was made into a dispersion by using beads in a sand mill (1/4 Gallon Sand Grinder Mill, 65 manufactured by Imex) to obtain a solid fine grain dispersion of the base precursor having an average particle diameter of  $0.2 \mu\text{m}$ .

83

## (Preparation of Solid Fine Grain Dispersion of Dye)

The cyanine dye compound (9.6 g) and sodium p-alkylbenzenesulfonate (5.8 g) were mixed with distilled water (305 ml), and the mixture was made into a dispersion by using beads in a sand mill (1/4 Gallon Sand Grinder Mill, manufactured by Imex) to obtain a solid fine grain dispersion of the dye having an average particle diameter of 0.2  $\mu\text{m}$ .

## (Preparation of Coating Solution for Antihalation Layer)

Gelatin (17 g), polyacrylamide (9.6 g), the aforementioned solid fine grain dispersion of base precursor (70 g), the aforementioned solid fine grain dispersion of dye (56 g), polymethyl methacrylate microparticles (average particle diameter of 6.5  $\mu\text{m}$ , 1.5 g), sodium polyethylenesulfonate (2.2 g), a 1 wt % aqueous solution of a coloring dye compound (0.2 g) and  $\text{H}_2\text{O}$  (844 ml) were mixed to prepare a coating solution for antihalation layer.

## (Preparation of Coating Solution for Protective Layer)

In a container kept at 40° C., gelatin (50 g), sodium polystyrenesulfonate (0.2 g), N,N-ethylenabis (vinylsulfonacetamide) (2.4 g), sodium t-octylphenoxyethoxyethanesulfonate (1 g), benzisothisazolinone (30 mg),  $\text{C}_8\text{F}_{17}\text{SO}_3\text{K}$  (32 mg),  $\text{C}_8\text{F}_{17}\text{SO}_2\text{N}(\text{C}_3\text{H}_7)$  ( $\text{CH}_2\text{CH}_2\text{O}_2$ )<sub>4</sub>( $\text{CH}_2$ )<sub>4</sub>— $\text{SO}_3\text{Na}$  (64 mg) and water (950 ml) were mixed to form a coating solution for protective layer.

The compounds used for Example 1 are shown below.

## Surface active agent 1



## Spectral sensitizing dye 1



## Tellurium compound



## Base precursor compound



US 6,376,166 B1

84

-continued



## &lt;&lt;Production of Heat-developable Photosensitive Material&gt;&gt;

On the aforementioned support having an undercoat layer, the coating solution for antihalation layer and the coating solution for protective layer were simultaneously applied as stacked layers so that the applied solid content amount of the solid fine grain dye in the antihalation layer should be 0.04 g/ $\text{m}^2$ , and the applied amount of gelatin in the protective layer should be 1 g/ $\text{m}^2$ , and dried to form an antihalation backing layer. Then, on the surface opposite to the back surface, an emulsion layer, intermediate layer, first protective layer, and second protective layer were simultaneously applied in this order from the undercoat layer by the slide bead application method as stacked layers to form a heat-developable photosensitive material (Table 1). After the application on the back surface, the emulsion layer was applied without winding the material.

The application was performed at a speed of 160 m/min, and the gap between the tip of coating die and the support was set to be 0.18 mm. The pressure in the reduced pressure chamber was adjusted to be lower than the atmospheric pressure by 392 Pa. In the subsequent chilling zone, the material was blown with air showing a dry-bulb temperature of 18° C. and a wet-bulb temperature of 12° C. at an average wind speed of 7 m/second for 30 seconds to cool the coating solutions. Then, in the floating type drying zone in a coiled shape, the material was blown with drying air showing a dry-bulb temperature of 30° C. and a wet-bulb temperature of 18° C. at a blowing wind speed of 20 m/second at nozzles for 200 seconds to evaporate the solvents in the coating solutions.

The results of the following evaluation for each photosensitive material sample are shown in Table 1.

## &lt;&lt;Evaluation of Photographic Performance&gt;&gt;

Each photosensitive material was light-exposed by a 647 nm Kr laser sensitometer (maximum output: 500 mW) at an angle of 300 with respect to the normal, and treated at 120° C. for 15 seconds (development). The obtained image was evaluated by a densitometer. The measurement results were

evaluated as Dmax, fog (Dmin) and sensitivity (a reciprocal of the ratio of the exposure amount necessary for giving a density 1.0 higher than Dmin). The sensitivity was expressed by a relative value to the sensitivity of Heat-developable photosensitive material 101 shown in Table 1 that was taken as 100.

calcium bromide dihydrate (0.90 g), 2-butanone (580 g) and dimethylformamide (220 g) with stirring, and left for 3 hours. Then, a phenol compound of the present invention (each compound shown in Table 2, 160 g), Exemplary compound B-42 (2.1 g) as an ultrahigh contrast agent, a coupler compound (each compound shown in Table 2,

TABLE 1

| Heat-developable photographic material | Phenol compound | Coupler compound | Photographic performance |      |             |             |
|----------------------------------------|-----------------|------------------|--------------------------|------|-------------|-------------|
|                                        |                 |                  | Dmax                     | Fog  | Sensitivity | Note        |
| 101                                    | I-1             | Not added        | 4.5                      | 0.27 | 100         | Comparative |
| 102                                    | I-1             | A-104            | 4.4                      | 0.18 | 98          | Invention   |
| 103                                    | I-1             | A-202            | 4.4                      | 0.22 | 99          | Invention   |
| 104                                    | I-1             | A-301            | 4.5                      | 0.14 | 99          | Invention   |
| 105                                    | I-1             | A-402            | 4.4                      | 0.15 | 99          | Invention   |
| 106                                    | I-1             | A-409            | 4.4                      | 0.16 | 99          | Invention   |
| 107                                    | I-1             | A-506            | 4.4                      | 0.20 | 99          | Invention   |
| 108                                    | I-1             | A-602            | 4.5                      | 0.18 | 99          | Invention   |
| 109                                    | I-2             | A-903            | 4.5                      | 0.14 | 100         | Invention   |
| 110                                    | I-1             | A-1005           | 4.4                      | 0.15 | 100         | Invention   |
| 111                                    | I-2             | A-1012           | 4.4                      | 0.15 | 99          | Invention   |
| 112                                    | I-2             | A-1106           | 4.4                      | 0.16 | 101         | Invention   |
| 113                                    | I-2             | A-1206           | 4.4                      | 0.20 | 99          | Invention   |
| 114                                    | I-1             | A-1309           | 4.5                      | 0.18 | 99          | Invention   |
| 115                                    | I-3             | A-1405           | 4.5                      | 0.20 | 99          | Invention   |
| 116                                    | I-3             | A-1509           | 4.4                      | 0.21 | 99          | Invention   |

It can be seen that fog was suppressed in Heat-developable photosensitive materials 102-116 without degrading Dmax and sensitivity, as evaluated by using Heat-developable photosensitive materials 101 as a blank, which did not contain any coupler compound.

#### Example 2

##### (Preparation of Organic Acid Silver Salt Emulsion A)

Behenic acid (933 g) was added to water (12 l), and added with sodium hydroxide (48 g) and sodium carbonate (63 g) dissolved in water (1.5 l) while the mixture was maintained at 90° C. After the mixture was stirred for 30 minutes, the temperature of the mixture was lowered to 50° C., and the mixture was added with a 1 wt % N-bromosuccinimide aqueous solution (1.1 l), and then gradually added with a 17% silver nitrate aqueous solution (2.3 l) with stirring. Then, the temperature of the mixture was lowered to 35° C., and the mixture was added with a 2 wt % potassium bromide aqueous solutions (1.5 l) over 2 minutes with stirring, then stirred for 30 minutes, and added with a 1 wt % N-bromosuccinimide aqueous solution (2.4 l). This aqueous mixture was added with a 1.2 wt % polyvinyl acetate solution in butyl acetate (3300 g) with stirring, and then left stand for 10 minutes so that the mixture should be separated into two layers. Then, the aqueous layer was removed, and the remained gel was washed twice with water. The gel-like mixture of silver behenate and silver bromide was dispersed in a 2.6% solution of polyvinyl butyral (Denka Butyral, DENKI KAGAKU KOGYO K.K., #3000K) in 2-butanone (1800 g), and further dispersed with polyvinyl butyral (Butvar B-76, Monsanto Japan, 600 g) and isopropyl alcohol (300 g) to obtain an organic acid silver salt emulsion (acicular grains having an average short axis length of 0.05  $\mu\text{m}$ , an average long axis length of 1.2  $\mu\text{m}$  and a variation coefficient of 25%).

##### (Preparation of Coating Solution for Emulsion Layer A)

The organic acid silver salt emulsion obtained above was added with the reagents in following amounts per 1 mole of silver. At 25° C., the emulsion was added with Sensitization dye A (520 mg), Compound (C-1) (1.70 g), 4-chlorobenzophenone-2-carboxylic acid (C-2) (21.5 g),

<sup>30</sup> 1.0×10<sup>-2</sup> mol), a dye (C-3) (1.11 g), Sumidur N3500 (polyisocyanate, Sumitomo Bayer Urethane Co., Ltd., 6.45 g), Megafax F-176P (fluorinated surface active agent, 0.60 g, Dai-Nihon Ink Chemical Industry Co., Ltd.), 2-butanone (590 g) and methyl isobutyl ketone (10 g) were added with stirring.

##### <sup>35</sup> (Preparation of Coating Solution for Protective Layer for Emulsion Layer A)

CAB171-15S (cellulose acetate butyrate, 65 g, Eastman Chemical Products, Inc.), phthalazine (C-4) (5.6 g), tetrachlorophthalic acid (C-5) (1.91 g), 4-methylphthalic acid (C-6) (2.6 g), tetrachlorophthalic acid anhydride (C-7) (0.67 g), Megafax F-176P (0.36 g) and Sildex H31 (spherical silica having an average size of 3  $\mu\text{m}$ , 2 g, Dokai Chemical K.K.) were dissolved in 2-butanone (1050 g) and dimethylformamide (50 g).

##### <sup>45</sup> (Preparation of Support with Backing Layer)

Polyvinyl butyral (Denka Butyral #4000 2, 6 g, DENKI KAGAKU KOGYO K.K.), Sildex H121 (spherical silica having an average size of 12  $\mu\text{m}$ , 0.2 g, Dokai Chemical K.K.), Sildex H51 (spherical silica having an average size of 5  $\mu\text{m}$ , 0.2 g, Dokai Chemical K.K.) and Megafax F-176P (0.1g) were added to 2-propanol (64 g) with stirring, dissolved and mixed in the solvent. To this mixture, a mixed solution of Dye A (420 mg) dissolved in methanol (10 g) and acetone (20 g) and a solution of 3-isocyanatomethyl-3,5,5-trimethylhexyl isocyanate (0.8 g) dissolved in ethyl acetate (6 g) were added to form a coating solution.

On a polyethylene terephthalate film having moisture proof undercoat layers comprising polyvinylidene chloride on the both surfaces, the coating solution of back layer was applied in such an amount that an optical density at 780 nm <sup>55</sup> should be 0.7.

On the support prepared as described above, the coating solution for emulsion layer was applied in such an amount that a silver coating amount of 1.6 g/m<sup>2</sup> should be obtained, and then the coating solution for protective layer for emulsion layer was applied on the emulsion layer surface in such an amount that a dry thickness of 2.3  $\mu\text{m}$  should be obtained.

The compounds used for Example 2 are shown below.

### Sensitizing dye A



(C-1)



(C-2)



(C-3)



(C-4)



(C-6)



-continued  
Dye A



## (Evaluation of Photographic Performance)

Each heat-developable photosensitive material was light-exposed by a xenon flash light of an emission time of  $10^{-4}$  seconds through an interference filter having a peak at 780 nm and a step wedge, and treated at 117° C. for 20 seconds (development) and at 120° C. for 20 seconds. The obtained image was evaluated by a densitometer. The measurement results were evaluated as Dmax, fog (Dmin) and sensitivity (a reciprocal of the ratio of the exposure amount necessary for giving a density 1.5 higher than Dmin). The sensitivity was expressed by a relative value to the sensitivity of Heat-developable photosensitive material 201 shown in Table 2 that was taken as 100. The results are shown in Table 2.

20 containing silver nitrate (18.6 g) and an aqueous solution containing 1 mol/l of potassium bromide were added by the control double jet method over 6 minutes and 30 seconds while pAg was maintained at 7.7. Then, 476 ml of an aqueous solution containing silver nitrate (55.5 g) and an aqueous halogen salt solution containing 1 mol/l of potassium bromide were added by the control double jet method over 28 minutes and 30 seconds while pAg was maintained at 7.7. Then, the pH was lowered to cause coagulation precipitation to thereby effect desalting, Compound A (0.17 g) and deionized gelatin (23.7 g, calcium content: 20 ppm or less) were added, and pH and pAg were adjusted to 5.9 and 8.0, respectively. The grains obtained were cubic grains

25

30

35

TABLE 2

| Heat-developable photographic material | Phenol compound | Coupler compound | Photographic performance |      |             |             |
|----------------------------------------|-----------------|------------------|--------------------------|------|-------------|-------------|
|                                        |                 |                  | Dmax                     | Fog  | Sensitivity | Note        |
| 201                                    | I-1             | Not added        | 4.6                      | 0.26 | 100         | Comparative |
| 202                                    | I-1             | A-105            | 4.5                      | 0.18 | 98          | Invention   |
| 203                                    | I-1             | A-204            | 4.5                      | 0.21 | 100         | Invention   |
| 204                                    | I-1             | A-301            | 4.5                      | 0.13 | 99          | Invention   |
| 205                                    | I-1             | A-401            | 4.5                      | 0.13 | 99          | Invention   |
| 206                                    | I-1             | A-409            | 4.5                      | 0.14 | 99          | Invention   |
| 207                                    | I-1             | A-505            | 4.6                      | 0.20 | 99          | Invention   |
| 208                                    | I-1             | A-603            | 4.6                      | 0.17 | 98          | Invention   |
| 209                                    | I-2             | A-903            | 4.5                      | 0.13 | 99          | Invention   |
| 210                                    | I-1             | A-1005           | 4.6                      | 0.15 | 99          | Invention   |
| 211                                    | I-2             | A-1012           | 4.5                      | 0.14 | 98          | Invention   |
| 212                                    | I-2             | A-1106           | 4.5                      | 0.15 | 99          | Invention   |
| 213                                    | I-2             | A-1206           | 4.4                      | 0.21 | 99          | Invention   |
| 214                                    | I-1             | A-1309           | 4.5                      | 0.17 | 98          | Invention   |
| 215                                    | I-3             | A-1405           | 4.6                      | 0.19 | 99          | Invention   |
| 216                                    | I-3             | A-1509           | 4.5                      | 0.22 | 99          | Invention   |

It can be seen that, even in the heat-developable photosensitive materials containing an ultrahigh contrast agent, the photosensitive materials 202-216, fog was more suppressed compared with the comparative photosensitive material 201.

Example 3  
<<Preparation of Silver Halide Emulsion>>  
(Emulsion A)

In 700 ml of water, phthalized gelatin (11 g), potassium bromide (30 mg) and sodium benzenethiosulfonate (10 mg) were dissolved. After the solution was adjusted to pH 5.0 at a temperature of 55° C., 159 ml of an aqueous solution

55 having an average grain size of 0.11  $\mu\text{m}$ , a variation coefficient of the projected area of 8% and a [100] face ratio of 93%.

The temperature of the silver halide grains obtained as described above was raised to 60° C., and added with 60 sodium benzenethiosulfonate (76  $\mu\text{mol}$  per mole of silver). After 3 minutes, sodium thiosulfate (154  $\mu\text{mol}$  per mole of silver) was further added, and then the grains were ripened for 100 minutes.

Then, Sensitization Dye B and Compound B were added 65 in amounts of  $6.4 \times 10^{-4}$  mol and  $6.4 \times 10^{-3}$  mol, respectively, per mole of silver halide with stirring while the emulsion is maintained at 40° C. After 20 minutes, the emulsion was

quenched to 30° C. to complete the preparation of Silver halide emulsion A.

<<Preparation of Organic Acid Silver Salt Dispersion>>  
(Organic Acid Silver Salt A)

Arachic acid (6.1 g), behenic acid (37.6 g), distilled water (700 ml), tert-butanol (70 ml) and 1 N aqueous NaOH solution (123 ml) were mixed, allowed to react at 75° C. for 1 hour with stirring, and cooled to 65° C. Then, 112.5 ml of an aqueous solution containing silver nitrate (22 g) was added to the mixture over 45 seconds. The mixture was left as it was for 5 minutes, and then the temperature was lowered to 30° C. Subsequently, the solid content was separated by suction filtration, and washed with water until the conductivity of the filtrate became 30  $\mu$ S/cm. The solid content obtained as described above was not dried but handled as a wet cake. To this wet cake corresponding to 100 g of dry solid content, 5 g of polyvinyl alcohol (trade name: PVA-205) and water were added to make the total amount of 500 g, and the resulting mixture was preliminarily dispersed in a homomixer.

Then, the preliminarily dispersed stock solution was treated three times in a dispersing machine (Microfluidizer M-110S-EH, manufactured by Microfluidex International Corporation, using G10Z interaction chamber) under a pressure controlled to be 1,750 kg/cm<sup>2</sup> to obtain Organic acid silver salt dispersion A. The organic acid silver salt grains contained in the organic acid silver salt dispersion obtained as described above were acicular grains having an average short axis length of 0.04  $\mu$ m, an average long axis length of 0.8  $\mu$ m and a variation coefficient of 30%. The grain size was measured by Master Sizer X manufactured by Malvern Instruments Ltd. During the cooling operation, a desired dispersion temperature was achieved by providing coiled heat exchangers fixed before and after the interaction chamber and controlling the temperature of the refrigerant. Thus, Organic acid silver salt A having a silver behenate content of 85 mol % was obtained.

<<Preparation of Solid Fine Grain Dispersion of Phenol Compound>>

To a phenol compound (each compound shown in Table 3, 70 g), MP Polymer (14 g, MP-203, produced by Kuraray Co., Ltd.) and water (266 ml) were added, and the mixture was thoroughly stirred to form a slurry. The resulting slurry was left for 3 hours. Then, 0.5-mm zirconia silicate beads (960 g) were prepared and put together with the slurry into a vessel. The contents in the vessel were dispersed in a dispersing machine (1/4G Sand Grinder Mill, manufactured by Imex) for 5 hours to prepare a reducing agent solid fine grain dispersion. In this dispersion, 80 wt % of the particles had a particle size of from 0.3 to 1.0  $\mu$ m.

<<Preparation of Solid Fine Grain Dispersion of Polyhalogenated Compound>>

To Polyhalogenated compound-P1 (30g), MP Polymer (5.0 g, MP-203, produced by Kuraray Co., Ltd.), Compound-C (0.21 g) and water (65 g) were added, and the mixture was thoroughly stirred to form a slurry. Then, the resulting slurry was put into a vessel together with 0.5-mm zirconia silicate beads (200 g). The contents in the vessel were dispersed in a dispersing machine (1/16G Sand Grinder Mill, manufactured by Imex) for 5 hours, then added with water (20 ml) and Compound-2 in such an amount that a concentration of 100 ppm should be obtained in the completed amount, and stirred for 10 minutes to prepare a solid fine grain dispersion. In this dispersion, the average particle diameter was 0.35  $\mu$ m, and the maximum particle diameter was 1.85  $\mu$ m.

Compound-P2 was also dispersed in the same manner as described above to obtain a solid fine grain dispersion.

<<Preparation of Solid Fine Grain Dispersion of Ultrahigh Contrast Agent>>

To the aforementioned Exemplary compound B-42 (10 g), polyvinyl alcohol (PVA-217, 2.5 g, Kraray Co., Ltd.) and water (87.5 g) were added and thoroughly mixed form a slurry, and a solid fine grain dispersion was prepared in the same manner as in the preparation of the reducing agent. In this dispersion, 80 wt % of the particles had a particle size of from 0.3 to 1.0  $\mu$ m.

<<Preparation of Coating Solution for Emulsion Layer>>

The binder, raw materials shown below and Silver halide emulsion A were added to the organic acid silver microcrystal dispersion prepared above in the indicated amounts per one mole of silver in the dispersion, and water was added to the mixture to form a coating solution for emulsion layer.

|                                                                                                                          |                                             |
|--------------------------------------------------------------------------------------------------------------------------|---------------------------------------------|
| Binder: LACSTAR 3307B<br>(SBR latex, produced by Dai-Nippon Ink & Chemicals, Inc., glass transition temperature: 17° C.) | 470 g as solid                              |
| Phenol compound                                                                                                          | 110 g as solid                              |
| Coupler compound<br>(each compound shown in Table 3)                                                                     | $1.5 \times 10^{-2}$ mol per mole of silver |
| 6-Methylbenzotriazole                                                                                                    | 1.35 g                                      |
| Polyvinyl alcohol (MP203, produced by Kuraray Co., Ltd.)                                                                 | 46 g                                        |
| Solid dispersion of Compound-P1                                                                                          | 44.8 g as Compound-P1                       |
| Solid dispersion of Compound-P2                                                                                          | 8.8 g as Compound-P2                        |
| 6-iso-Propylphthalazine                                                                                                  | 0.12 mol                                    |
| Dye B                                                                                                                    | 0.62 g                                      |
| Silver halide emulsion A                                                                                                 | 0.05 mol as Ag                              |
| Ultrahigh contrast agent<br>(solid dispersion of Exemplary compound B-42)                                                | 8.5 g as B-42                               |

<<Preparation of Coating Solution for Protective Layer for Emulsion Layer>>

A polymer latex containing 27.5 wt % of solid content (copolymer of methyl methacrylate/styrene/2-ethylhexyl acrylate/2-hydroxyethyl methacrylate/acrylic acid=59/9/26/5/1, glass transition temperature of 55° C., 109 g) was added with water (3.75 g), benzyl alcohol (4.5 g) as a film-forming aid, Compound D (0.45 g), Compound E (0.125 g), Compound F (1.70 g) and polyvinyl alcohol (PVA-217, Kuraray Co., Ltd., 0.285 g) and further added with water to a total amount of 150 g to form a coating solution.

<<Preparation of PET Support with Backing Layer and Undercoat Layer>>

(1) Support

PET having IV (intrinsic viscosity) of 0.66 (measured in phenol/tetrachloroethane=6/4 (weight ratio) at 25° C.) was obtained by using terephthalic acid and ethylene glycol in a conventional manner. The product was pelletized, dried at 130° C. for 4 hours, melted at 300° C., then extruded from a T-die and rapidly cooled to form an unstretched film having a thickness of 120  $\mu$ m after thermal fixation.

The film was stretched along the longitudinal direction by 3.3 times using rollers of different peripheral speeds, and then stretched along the transverse direction by 4.5 times using a tenter. The temperatures used for these operations were 110° C. and 130° C., respectively. Then, the film was subjected to thermal fixation at 240° C. for 20 seconds, and relaxed by 4% along the transverse direction at the same temperature. Then, the chuck of the tenter was released, the both edges of the film were knurled, and the film was rolled up at 4.8 kg/cm<sup>2</sup>. Thus, a roll of a film having a width of 2.4 m, length of 3500 m, and thickness of 120  $\mu$ m was obtained.

-continued

|                                                                                                                                                      |                                                   |
|------------------------------------------------------------------------------------------------------------------------------------------------------|---------------------------------------------------|
| <u>(2) Undercoat layer (a)</u>                                                                                                                       |                                                   |
| Polymer latex 1 (styrene/butadiene/hydroxyethyl methacrylate/divinylbenzene = 67/30/2.5/0.5 (% by weight))                                           | 160 g/m <sup>2</sup>                              |
| 2,4-Dichloro-6-hydroxy-s-triazine                                                                                                                    | 4 mg/m <sup>2</sup>                               |
| Matting agent (polystyrene, average diameter; 2.4 $\mu$ m)                                                                                           | 3 mg/m <sup>2</sup>                               |
| <u>(3) Undercoat layer (b)</u>                                                                                                                       |                                                   |
| Alkali-treated gelatin (Ca <sup>2+</sup> content; 30 ppm, jelly strength; 230 g)                                                                     | 50 mg/m <sup>2</sup>                              |
| Dye B                                                                                                                                                | Amount affording optical density of 1.0 at 780 nm |
| <u>(4) Electroconductive layer</u>                                                                                                                   |                                                   |
| Julimer ET-410 (Nihon Junyaku Co.)                                                                                                                   | 96 mg/m <sup>2</sup>                              |
| Gelatin                                                                                                                                              | 50 mg/m <sup>2</sup>                              |
| Compound A                                                                                                                                           | 0.2 mg/m <sup>2</sup>                             |
| Polyoxyethylene phenyl ether                                                                                                                         | 10 mg/m <sup>2</sup>                              |
| Sumitex Resin M-3 (water-soluble melamine resin, Sumitomo Chemical Co., Ltd.)                                                                        | 18 mg/m <sup>2</sup>                              |
| Dye B                                                                                                                                                | Amount affording optical density of 1.0 at 780 nm |
| SnO <sub>2</sub> /Sb (weight ratio: 9/1, acicular grains, short axis/long axis = 20–30, Ishihara Sangyo Kaisha, Ltd.)                                | 120 mg/m <sup>2</sup>                             |
| Matting agent (Polymethyl methacrylate, average particle size: 5 $\mu$ m)                                                                            | 7 mg/m <sup>2</sup>                               |
| <u>(5) Protective layer</u>                                                                                                                          |                                                   |
| Polymer latex 2 (copolymer of methyl methacrylate/styrene/2-ethylhexyl acrylate/2-hydroxyethylmethacrylate/acrylic acid = 59/9/26/5/1 (% by weight)) | 1000 mg/m <sup>2</sup>                            |
| Polystyrenesulfonate (molecular weight: 1000–5000)                                                                                                   | 2.6 mg/m <sup>2</sup>                             |
| Cellosol 524 (Chukyo Yushi Co., Ltd.)                                                                                                                | 30 mg/m <sup>2</sup>                              |
| Sumitex Resin N-3                                                                                                                                    | 218 mg/m <sup>2</sup>                             |

10 On one side of the support, Undercoat layer (a) and Undercoat layer (b) were successively coated and dried at 180° C. for 4 minutes. Subsequently, on the surface opposite to the surface coated with Undercoat layer (a) and Undercoat layer (b), an electroconductive layer and a protective layer 15 were successively coated and dried at 180° C. for 30 seconds to prepare a PET support with backing/undercoat layers.

20 The PET support with backing/undercoat layers obtained  
 21 as described above was introduced into a heat treatment  
 22 zone set at 150° C. and having a total length of 30 m, and  
 23 subjected to spontaneous transportation at a tension of 1.4  
 24 kg/cm<sup>2</sup> and a transportation speed of 20 m/minute. Then, the  
 25 support was passed through a zone at 40° C. for 15 seconds,  
 and taken up at a take-up tension of 10 kg/cm<sup>2</sup>.

## <<Preparation of Heat-developable Photosensitive Material>>

On the undercoat layer of the PET support with backing/undercoat layers, the aforementioned coating solution for emulsion layer was coated to give a coated silver amount of 1.6 g/m<sup>2</sup>. The coating solution for protective layer for emulsion layer was further coated on the emulsion layer so that the coated polymer latex solid amount of the protective layer should be 2.0 g/m<sup>2</sup> as a solid amount.

The compounds used for Example 3 are shown below.

### Sensitizing dye B





-continued  
Compound A



Compound C



Compound P-2



Dye B

Dye D



Dye F



Dye E

<<Evaluation of Photographic Performance>>  
(Light Exposure)

Each of the obtained heat-developable photosensitive materials was exposed by a xenon flash light of an emission time of  $10^{-6}$  seconds through an interference filter having a peak at 780 nm and a step wedge.  
(Heat Development)

The light-exposed heat-developable photosensitive material was heat-developed by using a heat-developing apparatus as shown in FIG. 1, in which the roller surface material was composed of silicone rubber, and the flat surface consisted of Teflon non-woven fabric. The heat development was performed at a carrying speed of 20 mm/second in the

45 preheating section at 90–100° C. for 15 seconds, in the heat developing section at 120° C. for 20 seconds and in the slow cooling section for 15 seconds. The temperature precision as for the transverse direction was  $\pm 1^\circ$  C.  
(Evaluation of Photographic Performance)

50 The obtained image was evaluated by Macbeth TD904 densitometer (visible density). The measurement results were evaluated as Dmax, fog (Dmin) and sensitivity (a reciprocal of the ratio of the exposure amount necessary for giving a density 1.5 higher than Dmin). The sensitivity was expressed by a relative value to the sensitivity of Heat-developable photosensitive material 301 that was taken as 100. The results are shown in Table 3.

TABLE 2

| Heat-developable photographic material | Phenol compound | Coupler compound | Photographic performance |      |             |             | Note |
|----------------------------------------|-----------------|------------------|--------------------------|------|-------------|-------------|------|
|                                        |                 |                  | Dmax                     | Fog  | Sensitivity |             |      |
| 301                                    | I-1             | Not added        | 4.6                      | 0.29 | 100         | Comparative |      |
| 302                                    | I-1             | A-105            | 4.6                      | 0.17 | 98          | Invention   |      |
| 303                                    | I-1             | A-209            | 4.5                      | 0.21 | 99          | Invention   |      |

TABLE 2-continued

| Heat-developable photographic material | Phenol compound | Coupler compound | Photographic performance |      |             |           |
|----------------------------------------|-----------------|------------------|--------------------------|------|-------------|-----------|
|                                        |                 |                  | Dmax                     | Fog  | Sensitivity | Note      |
| 304                                    | I-1             | A-302            | 4.6                      | 0.12 | 100         | Invention |
| 305                                    | I-1             | A-403            | 4.5                      | 0.13 | 99          | Invention |
| 306                                    | I-1             | A-409            | 4.5                      | 0.13 | 99          | Invention |
| 307                                    | I-1             | A-506            | 4.5                      | 0.20 | 99          | Invention |
| 308                                    | I-1             | A-605            | 4.6                      | 0.18 | 98          | Invention |
| 309                                    | I-2             | A-903            | 4.4                      | 0.14 | 100         | Invention |
| 310                                    | I-1             | A-1005           | 4.4                      | 0.15 | 100         | Invention |
| 311                                    | I-2             | A-1012           | 4.5                      | 0.15 | 99          | Invention |
| 312                                    | I-2             | A-1106           | 4.5                      | 0.16 | 100         | Invention |
| 313                                    | I-2             | A-1206           | 4.5                      | 0.20 | 99          | Invention |
| 314                                    | I-1             | A-1309           | 4.5                      | 0.18 | 99          | Invention |
| 315                                    | I-3             | A-1405           | 4.5                      | 0.20 | 99          | Invention |
| 316                                    | I-3             | A-1509           | 4.4                      | 0.21 | 99          | Invention |

Excellent photographic performance was obtained in the heat-developable photosensitive materials of the present invention in the presence of an ultrahigh contrast agent.

What is claimed is:

1. A heat-developable photosensitive material which comprises, on the same side of a support, at least (a) a photosensitive silver halide, (b) a reducible silver salt, (c) a phenol compound represented by the following formula (1), (d) a binder, and (e) a two or four equivalent coupler compound:



wherein V<sup>1</sup> to V<sup>6</sup> each independently represent a hydrogen atom or a functional group; L represents a bridging group selected from the group consisting of —CH(V<sup>9</sup>)— or —S—; V<sup>9</sup> represents a hydrogen atom or a functional group.

2. The heat-developable photosensitive material according to claim 1, wherein V<sup>1</sup> to V<sup>8</sup> each independently represent a hydrogen atom or an alkyl group.

3. The heat-developable photosensitive material according to claim 1, wherein L represents —CH(V<sup>9</sup>)— and V<sup>9</sup> represents a hydrogen atom, an alkyl group, an alkenyl group, an aryl group, hydroxyl group, mercapto group or an alkylthio group.

4. The heat-developable photosensitive material according to claim 1, wherein the phenol compound represented by the formula (1) is contained in an amount of 5 to 500 mmol per mole of silver present in the heat-developable photosensitive material.

5. The heat-developable photosensitive material according to claim 4, wherein the phenol compound represented by the formula (1) is contained in an amount of 10 to 400 mmol per mole of silver present in the heat-developable photosensitive material.

6. The heat-developable photosensitive material according to claim 1, wherein the phenol compound represented by the formula (1) is contained in a layer containing the silver halide or a layer adjacent thereto.

7. The heat-developable photosensitive material according to claim 1, wherein the coupler compound is selected from the group consisting of one or more of compounds represented by the following formulae (2) to (14):



(2)



(3)



(4)



(5)



(6)

-continued



-continued

(14)



(7) 5 10 wherein X<sup>1</sup> to X<sup>15</sup> each independently represent a hydrogen atom or a functional group in the formulae (2) to (14); R<sup>1</sup> and R<sup>2</sup> each independently represent an electron withdrawing group in the formula (2); R<sup>3</sup> to R<sup>28</sup> each independently represent a hydrogen atom or a functional group in the formulae (3) to (14); and q represents an integer of 0-4.

(8) 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770 9775 9780 9785 9790 9795 9800 9805 9810 9815 9820 9825 9830 9835 9840 9845 9850 9855 9860 9865 9870 9875 9880 9885 9890 9895 9900 9905 9910 9915 9920 9925 9930 9935 9940 9945 9950 9955 9960 9965 9970 9975 9980 9985 9990 9995 9999 10000 10005 10010 10015 10020 10025 10030 10035 10040 10045 10050 10055 10060 10065 10070 10075 10080 10085 10090 10095 10100 10105 10110 10115 10120 10125 10130 10135 10140 10145 10150 10155 10160 10165 10170 10175 10180 10185 10190 10195 10200 10205 10210 10215 10220 10225 10230 10235 10240 10245 10250 10255 10260 10265 10270 10275 10280 10285 10290 10295 10300 10305 10310 10315 10320 10325 10330 10335 10340 10345 10350 10355 10360 10365 10370 10375 10380 10385 10390 10395 10400 10405 10410 10415 10420 10425 10430 10435 10440 10445 10450 10455

**101**

18. The heat-developable photosensitive material according to claim 17, wherein the ultrahigh contrast agent is selected from the group consisting of one or more of compounds represented by the following formulae (17) to (19):



(17)

wherein in the formula (17),  $R^{1a}$ ,  $R^{2a}$  and  $R^{3a}$  each independently represents a hydrogen atom or a functional group, and  $Z$  represents an electron withdrawing group or a silyl group;  $R^{1a}$  together with  $Z$ ,  $R^{2a}$  together with  $R^{3a}$ ,  $R^{1a}$  together with  $R^{2a}$ , or  $R^{3a}$  together with  $Z$  may combine with each other to form a ring structure; in the formula (18),  $R^{4a}$  represents a functional group; and in the formula (19),  $X$  and  $Y$  independently represent a hydrogen atom or a functional group,  $A$  and  $B$  independently represent an alkoxy group, an alkylthio group, an alkylamino group, an aryloxy group, an arylthio group, an anilino group, a heterocyclyloxy group, a heterocyclithio group or a heterocyclamino group, and  $X$  together with  $Y$ , or  $A$  together with  $B$  may be combined with each other to form a ring structure.

(18)

10

15

20

**102**

-continued

(19)



\* \* \* \* \*